



US006027869A

# United States Patent [19]

Maskasky et al.

[11] Patent Number: 6,027,869

[45] Date of Patent: Feb. 22, 2000

[54] **PHOTOGRAPHIC ELEMENTS CONTAINING LIGHT SCATTERING PARTICLES**

[75] Inventors: **Joe E. Maskasky; Kenneth J. Reed; Victor P. Scaccia; James A. Friday**, all of Rochester, N.Y.

[73] Assignee: **Eastman Kodak Company**, Rochester, N.Y.

[21] Appl. No.: 09/213,644

[22] Filed: Dec. 17, 1998

[51] Int. Cl.<sup>7</sup> ..... G03C 1/10; G03C 1/08; G03C 1/035

[52] U.S. Cl. ..... 430/567; 430/569; 430/639; 430/640; 430/599; 430/600; 430/603; 430/950

[58] Field of Search ..... 430/567, 569, 430/639, 640, 950, 599, 600, 603

## [56] References Cited

### U.S. PATENT DOCUMENTS

|           |         |               |       |         |
|-----------|---------|---------------|-------|---------|
| 4,439,520 | 3/1984  | Kofron et al. | ..... | 430/434 |
| 5,604,085 | 2/1997  | Maskasky      | ..... | 430/567 |
| 5,620,840 | 4/1997  | Maskasky      | ..... | 430/567 |
| 5,667,955 | 9/1997  | Maskasky      | ..... | 430/567 |
| 5,691,131 | 11/1997 | Maskasky      | ..... | 430/639 |
| 5,733,718 | 3/1998  | Maskasky      | ..... | 430/639 |
| 5,747,235 | 5/1998  | Farid et al.  | ..... | 430/598 |
| 5,747,236 | 5/1998  | Farid et al.  | ..... | 430/583 |

## FOREIGN PATENT DOCUMENTS

0786692 7/1997 European Pat. Off. ..... G03C 1/16

## OTHER PUBLICATIONS

Research Disclosure, vol. 389, Sep. 1996, Item 38957, I., II., IV., V., and X.

Primary Examiner—Mark F. Huff  
Attorney, Agent, or Firm—Carl O. Thomas

## [57] ABSTRACT

A photographic element is disclosed having at least one emulsion layer comprised of (a) radiation-sensitive silver halide grains, (b) sensitizer for the radiation-sensitive silver halide grains, (c) hydrophilic colloid vehicle, including peptizer for the radiation-sensitive silver halide grains, and (d) light scattering particles, wherein (a) the radiation-sensitive silver halide grains include tabular grains (1) having an aspect ratio of at least 2.0, (2) having {111} major faces, (3) containing greater than 50 mole percent bromide, based on silver, and (4) accounting for greater than 50 percent total grain projected area, (b) the sensitizer includes a fragmentable electron donating sensitizer, (c) the peptizer is a water dispersible cationic starch, and (d) the light scattering particles have aspect ratios of less than 1.5 and can be dissolved for removal from the emulsion layer. The photographic elements exhibit enhanced imaging speed and can be employed for color or black-and-white photographic imaging.

16 Claims, No Drawings

## PHOTOGRAPHIC ELEMENTS CONTAINING LIGHT SCATTERING PARTICLES

### FIELD OF THE INVENTION

The invention relates to silver halide photography. More specifically, the invention relates to radiation-sensitive emulsions and photographic elements useful in silver halide photography.

### BACKGROUND OF THE INVENTION

The most widely used forms of photographic elements are those that contain one or more silver halide emulsions. Silver halide emulsions are usually prepared by precipitating silver halide in the form of discrete grains (microcrystals) in an aqueous medium. An organic peptizer is incorporated in the aqueous medium to disperse the grains. Varied forms of hydrophilic colloids are known to be useful as peptizers, but the overwhelming majority of silver halide emulsions employ gelatino-peptizers. A summary of conventional peptizers, including gelatino-peptizers, is provided by *Research Disclosure*, Vol. 389, September 1996, Item 38957, II. Vehicles, vehicle extenders, vehicle-like addenda and vehicle related addenda, A. Gelatin and hydrophilic colloid peptizers. *Research Disclosure* is published by Kenneth Mason Publications, Ltd., Dudley House, 12 North St., Emsworth, Hampshire PO10 7DQ, England. The term "vehicle" includes both the peptizer used to disperse silver halide grains as they are being formed and the binder used in coating emulsion and processing solution penetrable layers of photographic elements. Gelatin and gelatin derivatives are commonly employed to perform the functions of both peptizer and binder.

The characteristic that is primarily responsible for the dominance of silver halide photography is the image amplification capability of silver halide grains. During imagewise exposure of a silver halide photographic element, incident photons are absorbed by the silver halide grains. When a photon is absorbed, an electron in the silver halide crystal lattice structure of a grain is promoted from a valence band energy level to a higher, conduction band energy level at which it is capable of migrating within the crystal lattice of the grain. When a few conduction band electrons are captured by crystal lattice silver ions in close proximity, a cluster of  $\text{Ag}^{\circ}$  atoms is created, commonly referred to as a latent image site. The latent image site of a grain is capable of catalyzing the overall reduction of silver ions in the grain to  $\text{Ag}^{\circ}$ , a huge amplification of the few original  $\text{Ag}^+$  reductions to  $\text{Ag}^{\circ}$  created by imagewise exposure. An imagewise exposed silver halide emulsion is brought into contact with a developer to produce a viewable image. A developer is an aqueous solution containing a developing agent, a reducing agent capable of selectively reducing latent image bearing silver halide grains to  $\text{Ag}^{\circ}$ . Contacting a photographic element with aqueous solutions, including a developer, to produce a viewable image is referred to as photographic processing.

Although many factors come into play in obtaining desirable photographic images, one of the most fundamental is the speed of the photographic element employed. While silver halide photography with its internal amplification mechanism exhibits much higher photographic speeds than other imaging systems, the search for higher photographic speeds in silver halide photography has continued since its inception to the present time, a time period of well over a century. The speed of a photographic element is measured by exposing sample portions of the element at differing

levels and then correlating image density following photographic processing. By plotting image density ( $D$ ) as an ordinate against the log of exposure ( $E$ ) in lux-seconds, a characteristic curve is generated. The characteristic curve typically contains a portion that exhibits no change in density (minimum density or  $D_{min}$ ) as a function of exposure transitioning with increased exposures to a portion in which density increases as a function of increased exposure, often resulting in a linear characteristic curve segment (i.e.,  $\Delta D/\Delta \log E$  remains constant) transitioning with still higher exposures to a portion in which further exposure does not increase density (maximum density or  $D_{max}$ ). Photographic element speeds are usually reported as differences in  $\log E$  required to produce the same density in compared elements.

Silver halide emulsions possess a native sensitivity to light having wavelengths ranging from the ultraviolet into the blue region of the visible spectrum. Spectral sensitizing dyes are adsorbed to the silver halide grain surfaces to extend sensitivity to longer wavelength portions of the spectrum. A summary of spectral sensitizing dyes is provided by *Research Disclosure*, Item 38957, cited above, V. Spectral sensitization and desensitization, A. Sensitizing Dyes. The function of a spectral sensitizer is to capture for latent image formation a photon of a wavelength the silver halide grain cannot itself capture.

To increase the speed of silver halide emulsions independent of spectral sensitization, the grain surfaces are treated with chemical sensitizers. A summary of chemical sensitizers is provided by *Research Disclosure*, Item 38957, cited above, IV. Chemical sensitization.

It has been recently recognized that a further enhancement in photographic speed can be realized by associating with the silver halide grain surfaces a fragmentable electron donating (FED) sensitizer. While no proof of the mechanism of FED sensitization has yet been generated, one plausible explanation is as follows: When, as noted above, photon capture within a grain results in electron promotion from a valence shell to a conduction energy band, a common loss factor is recombination. That is, the promoted electron simply returns to a hole in the valence shell, created by promotion to the conduction band of the same or another electron. When recombination occurs, the energy of the captured photon is dissipated without contributing to latent image formation. It is believed that the FED sensitizer reduces recombination by donating an electron to fill the hole created by photon capture. Thus, fewer conduction band electrons return to hole sites in valence bands and more electrons are available to participate in latent image formation.

When the FED sensitizer donates an electron to a silver halide grain, it fragments, creating a cation and a free radical. The free radical is a single atom or compound that contains an unpaired valence shell electron and is for that reason highly unstable. If the oxidation potential of the free radical is equal to or more negative than  $-0.7$  volt, the free radical immediately upon formation injects a second electron into the grain to eliminate its unpaired valence shell electron. When the free radical also donates an electron to the grain, it is apparent that absorption of a single photon in the grain has promoted an electron to the conduction band, stimulated the FED sensitizer to donate an electron to fill the hole left behind by the promoted electron, thereby reducing hole-electron recombination, and injected a second electron. Thus, the FED sensitizer contributes one or two electrons to the silver grain that contribute directly or indirectly to latent image formation.

FED sensitizers and their utilization for increasing photographic speed are disclosed in Farid et al U.S. Pat. Nos.

5,747,235 and 5,7547,236, and in the following commonly assigned filings: Lenhard et al U.S. Ser. No. 08/739,911, filed Oct. 30, 1996, and Gould et al U.S. Ser. No. 09/118,536, Farid et al U.S. Ser. No. 09/118,552, and Adin et al U.S. Ser. No. 09/118,714, each filed Jun. 25, 1998.

A dramatic increase in photographic speeds in silver halide photography began with the introduction of tabular grain emulsions into silver halide photographic products in 1982. A tabular grain is one which has two parallel major faces that are clearly larger than any other crystal face and which has an aspect ratio of at least 2. The term "aspect ratio" is the ratio of the equivalent circular diameter (ECD) of the grain divided by its thickness (the distance separating the major faces). Tabular grain emulsions are those in which tabular grains account for greater than 50 percent of total grain projected area. Kofron et al U.S. Pat. No. 4,439,520 illustrates the first chemically and spectrally sensitized high aspect ratio (average aspect ratio >8) tabular grain emulsions. In their most commonly used form tabular grain emulsions contain tabular grains that have major faces lying in {111} crystal lattice planes and contain greater than 50 mole percent bromide, based on silver. A summary of tabular grain emulsions is contained in *Research Disclosure*, Item 38957, cited above, I. Emulsion grains and their preparation, B. Grain morphology, particularly sub-paragraphs (1) and (3).

The use of cationic starch as a peptizer for the precipitation of high bromide {111} tabular grain emulsions is taught by Maskasky U.S. Pat. Nos. 5,604,085, 5,620,840, 5,667, 955, 5,691,131, and 5,733,718. Oxidized cationic starches are advantageous in exhibiting lower levels of viscosity than gelatino-peptizers. This facilitates mixing. Under comparable levels of chemical sensitization higher photographic speeds can be realized using cationic starch peptizers. Alternatively, speeds equal to those obtained using gelatino-peptizers can be achieved at lower precipitation and/or sensitization temperatures, thereby avoiding unwanted grain ripening.

It has been proposed from time to time to incorporate light scattering particles into silver halide emulsion layers to increase their imaging speed. Materials of this type are disclosed in *Research Disclosure*, Item 38957, VIII. Absorbing and scattering materials, A. Reflective materials.

#### RELATED APPLICATIONS

Applicants' concurrently filed, commonly assigned patent application U.S. Ser. No. 09/213,739, titled PHOTOGRAPHIC EMULSIONS AND ELEMENTS OF INCREASED SENSITIVITY, (hereinafter referred to as Application I) is directed to a photographic emulsion comprised of (a) radiation-sensitive silver halide grains, (b) sensitizer for the silver halide grains, and (c) peptizer for the silver halide grains wherein (a) the radiation-sensitive silver halide grains include tabular grains (1) having {111} major faces, (2) containing greater than 50 mole percent bromide, based on silver, and (3) accounting for greater than 50 percent total grain projected area, (b) the sensitizer includes a fragmentable electron donating sensitizers, and (c) the peptizer is a water dispersible cationic starch.

Applicants' concurrently filed, commonly assigned patent application U.S. Ser. No. 09/213,639, titled COLOR PHOTOGRAPHIC ELEMENTS OF INCREASED SENSITIVITY, (hereinafter referred to as Application II) is directed to a photographic recording element comprised of a support and at least one dye image forming layer unit containing (a) radiation-sensitive silver halide grains, (b)

sensitizer for the silver halide grains, (c) peptizer for the silver halide grains, (d) at least one dye image providing coupler, and (e) at least one dye image enhancing coupler, wherein (a) the radiation-sensitive silver halide grains include tabular grains (1) having {111} major faces, (2) containing greater than 50 mole percent bromide, based on silver, and (3) accounting for greater than 50 percent total grain projected area, (b) the sensitizer includes a fragmentable electron donating sensitizers, (c) the peptizer is a water dispersible cationic starch, (d) the dye image providing coupler is a coupler capable of reacting with oxidized primary amine color developing agent to form a dye image, and (e) the dye image enhancing coupler is a coupler capable of reacting with oxidized primary amine color developing agent to release an electron transfer agent.

Applicants' concurrently filed, commonly assigned patent application U.S. Ser. No. 09/213/766, titled COLOR PHOTOGRAPHIC ELEMENTS OF INCREASED SENSITIVITY CONTAINING ONE EQUIVALENT COUPLER, (hereinafter referred to as Application III) is directed to a photographic recording element comprised of a support and at least one dye image forming layer unit containing (a) radiation-sensitive silver halide grains, (b) sensitizer for the silver halide grains, (c) peptizer for the silver halide grains, and (d) at least one dye image providing coupler, wherein (a) the radiation-sensitive silver halide grains include tabular grains (1) having {111} major faces, (2) containing greater than 50 mole percent bromide, based on silver, and (3) accounting for greater than 50 percent total grain projected area, (b) the sensitizer includes a fragmentable electron donating sensitizers, (c) the peptizer is a water dispersible cationic starch, and (d) the dye image providing coupler is a one equivalent image dye-forming coupler.

#### SUMMARY OF THE INVENTION

In one aspect the invention is directed to a photographic element comprised of a support and coated on the support at least one emulsion layer comprised of (a) radiation-sensitive silver halide grains, (b) sensitizer for the radiation-sensitive silver halide grains, (c) organic hydrophilic colloid vehicle, including peptizer for the radiation-sensitive silver halide grains, and (d) light scattering particles, wherein (a) the radiation-sensitive silver halide grains include tabular grains (1) having an average aspect ratio of at least 2.0, (2) having {111} major faces, (3) containing greater than 50 mole percent bromide, based on silver, and (4) accounting for greater than 50 percent total grain projected area, (b) the sensitizer includes a fragmentable electron donating sensitizers, (c) the peptizer is a water dispersible cationic starch, and (d) the light scattering particles have aspect ratios of less than 1.5 and can be dissolved for removal from the emulsion layer.

In comparing high bromide {111} tabular grain emulsions precipitated in the presence of a cationic starch peptizer and sensitized with a fragmentable electron donating (FED) sensitizers with an otherwise similar emulsion that contains a gelatino-peptizer, the starch peptized emulsions have been observed to exhibit significantly higher speeds than the gelatin peptized emulsions. When the comparisons are repeated, but with the FED sensitizers removed, a relatively small speed advantage is observed for the starch peptized emulsions. The large speed advantage realized by FED sensitizers addition to starch peptized high bromide {111} tabular grain emulsions was entirely unexpected.

It has been observed further that when a starch peptized high bromide {111} tabular grain emulsion according to this

invention is treated with an oxidizing agent prior to FED sensitization, it exhibits minimum density levels near those attainable when a gelatino-peptizer is employed. Thus, the large speed advantage of the emulsions of the invention can be realized with little, if any, increase in minimum densities.

The light scattering particles impart an additional increase in speed. By choosing light scattering particles that can be dissolved for removal from the emulsion layer, minimum densities in the processed elements can be retained similar to those of comparable elements initially lacking the light scattering particles. When, as is preferred, the light scattering particles are removed during photographic processing, no increase in processing complexity is required to remove the particles.

#### DETAILED DESCRIPTION OF THE INVENTION

The present invention is generally applicable to cationic starch peptized high bromide {111} tabular grain emulsions. High bromide {111} tabular grain emulsions are those in which greater than 50 percent of total grain projected area is accounted for by tabular grains having {111} major faces and containing greater than 50 mole percent bromide, based on silver.

Any conventional water dispersible cationic starch can be employed as a peptizer. The term "starch" is employed to include both natural starch and modified derivatives, such as dextrinated, hydrolyzed, alkylated, hydroxyalkylated, acetylated or fractionated starch. The starch can be of any origin, such as corn starch, wheat starch, potato starch, tapioca starch, sago starch, rice starch, waxy corn starch or high amylose corn starch.

Starches are generally comprised of two structurally distinctive polysaccharides,  $\alpha$ -amylose and amylopectin. Both are comprised of  $\alpha$ -D-glucopyranose units. In  $\alpha$ -amylose the  $\alpha$ -D-glucopyranose units form a 1,4-straight chain polymer. The repeating units take the following form:



In amylopectin, in addition to the 1,4-bonding of repeating units, 6-position chain branching (at the site of the  $-\text{CH}_2\text{OH}$  group above) is also in evidence, resulting in a branched chain polymer. The repeating units of starch and cellulose are diastereoisomers that impart different overall geometries to the molecules. The  $\alpha$  anomer, found in starch and shown in formula I above, results in a polymer that is capable of crystallization and some degree of hydrogen bonding between repeating units in adjacent molecules, but not to the same degree as the  $\beta$  anomer repeating units of cellulose and cellulose derivatives. Polymer molecules formed by the  $\beta$  anomers show strong hydrogen bonding between adjacent molecules, resulting in clumps of polymer molecules and a much higher propensity for crystallization. Lacking the alignment of substituents that favors strong intermolecular bonding, found in cellulose repeating units, starch and starch derivatives are much more readily dispersed in water.

The water dispersible starches employed in the practice of the invention are cationic—that is, they contain an overall net positive charge when dispersed in water. Starches are conventionally rendered cationic by attaching a cationic substituent to the  $\alpha$ -D-glucopyranose units, usually by esterification or etherification at one or more free hydroxyl sites. Reactive cationogenic reagents typically include a primary, secondary or tertiary amino group (which can be subsequently protonated to a cationic form under the intended conditions of use) or a quaternary ammonium, sulfonium or phosphonium group.

To be useful as a peptizer the cationic starch must be water dispersible. Many starches disperse in water upon heating to temperatures up to boiling for a short time (e.g., 5 to 30 minutes). High sheer mixing also facilitates starch dispersion. The presence of cationic substituents increases the polar character of the starch molecule and facilitates dispersion. The starch molecules preferably achieve at least a colloidal level of dispersion and ideally are dispersed at a molecular level—i.e., dissolved.

The following teachings, the disclosures of which are here incorporated by reference, illustrate water dispersible cationic starches within the contemplation of the invention:

\*Rutenberg et al U.S. Pat. No. 2,989,520;

Meisel U.S. Pat. No. 3,017,294;

Elizer et al U.S. Pat. No. 3,051,700;

Aszlos U.S. Pat. No. 3,077,469;

Elizer et al U.S. Pat. No. 3,136,646;

\*Barber et al U.S. Pat. No. 3,219,518;

\*Mazzarella et al U.S. Pat. No. 3,320,080;

Black et al U.S. Pat. No. 3,320,118;

Caesar U.S. Pat. No. 3,243,426;

Kirby U.S. Pat. No. 3,336,292;

Jarowenko U.S. Pat. No. 3,354,034;

Caesar U.S. Pat. No. 3,422,087;

\*Dishburger et al U.S. Pat. No. 3,467,608;

\*Beaninga et al U.S. Pat. No. 3,467,647;

Brown et al U.S. Pat. No. 3,671,310;

Cescato U.S. Pat. No. 3,706,584;

Jarowenko et al U.S. Pat. No. 3,737,370;

\*Jarowenko U.S. Pat. No. 3,770,472;

Moser et al U.S. Pat. No. 3,842,005;

Tessler U.S. Pat. No. 4,060,683;

Rankin et al U.S. Pat. No. 4,127,563;

Huchette et al U.S. Pat. No. 4,613,407;

Blixt et al U.S. Pat. No. 4,964,915;

\*Tsai et al U.S. Pat. No. 5,227,481; and

\*Tsai et al U.S. Pat. No. 5,349,089.

It is preferred to employ an oxidized cationic starch. The starch can be oxidized before (\* patents above) or following the addition of cationic substituents. This is accomplished by treating the starch with a strong oxidizing agent. Both hypochlorite ( $\text{ClO}^-$ ) or periodate ( $\text{IO}_4^-$ ) have been extensively used and investigated in the preparation of commercial starch derivatives and preferred. While any convenient oxidizing agent counter ion can be employed, preferred counter ions are those fully compatible with silver halide emulsion preparation, such as alkali and alkaline earth cations, most commonly sodium, potassium or calcium.

When the oxidizing agent opens the  $\alpha$ -D-glucopyranose ring, the oxidation sites are usually at the 2 and 3 position carbon atoms forming the  $\alpha$ -D-glucopyranose ring. The 2 and 3 position



groups are commonly referred to as the glycol groups. The carbon-to-carbon bond between the glycol groups is replaced in the following manner:



where R represents the atoms completing an aldehyde group or a carboxyl group.

The hypochlorite oxidation of starch is most extensively employed in commercial use. The hypochlorite is used in small quantities to modify impurities in starch. Any modification of the starch at these low levels is minimal, at most affecting only the polymer chain terminating aldehyde groups, rather than the  $\alpha$ -D-glucopyranose repeating units themselves. At levels of oxidation that affect the  $\alpha$ -D-glucopyranose repeating units the hypochlorite affects the 2, 3 and 6 positions, forming aldehyde groups at lower levels of oxidation and carboxyl groups at higher levels of oxidation. Oxidation is conducted at mildly acidic and alkaline pH (e.g., >5 to 11). The oxidation reaction is exothermic, requiring cooling of the reaction mixture. Temperatures of less than 45° C. are preferably maintained. Using a hypobromite oxidizing agent is known to produce similar results as hypochlorite.

Hypochlorite oxidation is catalyzed by the presence of bromide ions. Since silver halide emulsions are conventionally precipitated in the presence of a stoichiometric excess of the halide to avoid inadvertent silver ion reduction (fogging), it is conventional practice to have bromide ions in the dispersing media of high bromide silver halide emulsions. Thus, it is specifically contemplated to add bromide ion to the starch prior to performing the oxidation step in the concentrations known to be useful in the high bromide {111} tabular grain emulsions—e.g., up to a pBr of 3.0.

Cescato U.S. Pat. No. 3,706,584, the disclosure of which is here incorporated by reference, discloses techniques for

- the hypochlorite oxidation of cationic starch. Sodium bromite, sodium chlorite and calcium hypochlorite are named as alternatives to sodium hypochlorite. Further teachings of the hypochlorite oxidation of starches is provided by the following: R. L. Whistler, E. G. Linke and S. Kazeniac, "Action of Alkaline Hypochlorite on Corn Starch Amylose and Methyl 4-O-Methyl-D-glucopyranosides", *Journal Amer. Chem. Soc.*, Vol. 78, pp. 4704-9 (1956); R. L. Whistler and R. Schweiger, "Oxidation of Amylopectin with Hypochlorite at Different Hydrogen Ion Concentrations", *Journal Amer. Chem. Soc.*, Vol. 79, pp. 6460-6464 (1957); J. Schmorak, D. Mezler and M. Lewin, "A Kinetic Study of the Mild Oxidation of Wheat Starch by Sodium Hypochlorite in the Alkaline pH Range", *Journal of Polymer Science*, Vol. XLIX, pp. 203-216 (1961); J. Schmorak and M. Lewin, "The Chemical and Physico-chemical Properties of Wheat Starch with Alkaline Sodium Hypochlorite", *Journal of Polymer Science: Part A*, Vol. 1, pp. 2601-2620 (1963); K. F. Patel, H. U. Mehta and H. C. Srivastava, "Kinetics and Mechanism of Oxidation of Starch with Sodium Hypochlorite", *Journal of Applied Polymer Science*, Vol. 18, pp. 389-399 (1974); R. L. Whistler, J. N. Bemiller and E. F. Paschall, *Starch: Chemistry and Technology*, Chapter X, Starch Derivatives: Production and Uses, II. Hypochlorite-Oxidized Starches, pp. 315-323, Academic Press, 1984; and O. B. Wurzburg, *Modified Starches: Properties and Uses*, III. Oxidized or Hypochlorite-Modified Starches, pp. 23-28 and pp. 245-246, CRC Press (1986). Although hypochlorite oxidation is normally carried out using a soluble salt, the free acid can alternatively be employed, as illustrated by M. E. McKillican and C. B. Purves, "Estimation of Carboxyl, Aldehyde and Ketone Groups in Hypochlorous Acid Oxystarches", *Can. J. Chem.*, Vol. 312-321 (1954). Periodate oxidizing agents are of particular interest, since they are known to be highly selective. The periodate oxidizing agents produce starch dialdehydes by the reaction shown in the formula (II) above without significant oxidation at the site of the 6 position carbon atom. Unlike hypochlorite oxidation, periodate oxidation does not produce carboxyl groups and does not produce oxidation at the 6 position. Mehlretter U.S. Pat. No. 3,251,826, the disclosure of which is here incorporated by reference, discloses the use of periodic acid to produce a starch dialdehyde which is subsequently modified to a cationic form. Mehlretter also discloses for use as oxidizing agents the soluble salts of periodic acid and chlorine. Further teachings of the periodate oxidation of starches is provided by the following: V. C. Barry and P. W. D. Mitchell, "Properties of Periodate-oxidized Polysaccharides. Part II. The Structure of some Nitrogen-containing Polymers", *Journal Amer. Chem. Soc.*, 1953, pp. 3631-3635; P. J. Borchert and J. Mirza, "Cationic Dispersions of Dialdehyde Starch I. Theory and Preparation", *Tappi*, Vol. 47, No. 9, pp. 525-528 (1964); J. E. McCormick, "Properties of Periodate-oxidized Polysaccharides. Part VII. The Structure of Nitrogen-containing Derivatives as deduced from a Study of Monosaccharide Analogues", *Journal Amer. Chem. Soc.*, pp. 2121-2127 (1966); and O. B. Wurzburg, *Modified Starches: Properties and Uses*, III. Oxidized or Hypochlorite-Modified Starches, pp. 28-29, CRC Press (1986). Starch oxidation by electrolysis is disclosed by F. F. Farley and R. M. Hixon, "Oxidation of Raw Starch Granules by Electrolysis in Alkaline Sodium Chloride Solution", *Ind. Eng. Chem.*, Vol. 34, pp. 677-681 (1942). Depending upon the choice of oxidizing agents employed, one or more soluble salts may be released during the oxidation step. Where the soluble salts correspond to or are

similar to those conventionally present during silver halide precipitation, the soluble salts need not be separated from the oxidized starch prior to silver halide precipitation. It is, of course, possible to separate soluble salts from the oxidized cationic starch prior to precipitation using any conventional separation technique. For example, removal of halide ion in excess of that desired to be present during grain precipitation can be undertaken. Simply decanting solute and dissolved salts from oxidized cationic starch particles is a simple alternative. Washing under conditions that do not solubilize the oxidized cationic starch is another preferred option. Even if the oxidized cationic starch is dispersed in a solute during oxidation, it can be separated using conventional ultrafiltration techniques, since there is a large molecular size separation between the oxidized cationic starch and soluble salt by-products of oxidation.

The carboxyl groups formed by oxidation take the form  $-\text{C}(\text{O})\text{OH}$ , but, if desired, the carboxyl groups can, by further treatment, take the form  $-\text{C}(\text{O})\text{OR}'$ , where  $\text{R}'$  represents the atoms forming a salt or ester. Any organic moiety added by esterification preferably contains from 1 to 6 carbon atoms and optimally from 1 to 3 carbon atoms.

The minimum degree of oxidation contemplated is that required to reduce the viscosity of the starch. It is generally accepted (see citations above) that opening an  $\alpha$ -D-glucopyranose ring in a starch molecule disrupts the helical configuration of the linear chain of repeating units which in turn reduces viscosity in solution. It is contemplated that at least one  $\alpha$ -D-glucopyranose repeating unit per starch polymer, on average, be ring opened in the oxidation process. As few as two or three opened  $\alpha$ -D-glucopyranose rings per polymer has a profound effect on the ability of the starch polymer to maintain a linear helical configuration. It is generally preferred that at least 1 percent of the glucopyranose rings be opened by oxidation.

A preferred objective is to reduce the viscosity of the cationic starch by oxidation to less than four times (400 percent of) the viscosity of water at the starch concentrations employed in silver halide precipitation. Although this viscosity reduction objective can be achieved with much lower levels of oxidation, starch oxidations of up to 90 percent of the  $\alpha$ -D-glucopyranose repeating units have been reported (Wurzburg, cited above, p. 29). A typical convenient range of oxidation ring-opens from 3 to 50 percent of the  $\alpha$ -D-glucopyranose rings.

The water dispersible cationic starch is present during the precipitation (during nucleation and grain growth or during grain growth) of the high bromide {111} tabular grains. Preferably precipitation is conducted by substituting the water dispersible cationic starch for all conventional gelatino-peptizers. In substituting the selected cationic starch peptizer for conventional gelatino-peptizers, the concentrations of the selected peptizer and the point or points of addition can correspond to those employed using gelatino-peptizers.

In addition, it has been unexpectedly discovered that emulsion precipitation can tolerate even higher concentrations of the selected peptizer. For example, it has been observed that all of the selected peptizer required for the preparation of an emulsion through the step of chemical sensitization can be present in the reaction vessel prior to grain nucleation. This has the advantage that no peptizer additions need be interjected after tabular grain precipitation has commenced. It is generally preferred that from 1 to 500 grams (most preferably from 5 to 100 grams) of the selected peptizer per mole of silver to be precipitated be present in the reaction vessel prior to tabular grain nucleation.

At the other extreme, it is, of course, well known, as illustrated by Mignot U.S. Pat. No. 4,334,012, here incorporated by reference, that no peptizer is required to be present during grain nucleation, and, if desired, addition of the selected peptizer can be deferred until grain growth has progressed to the point that peptizer is actually required to avoid tabular grain agglomeration.

The procedures for high bromide {111} tabular grain emulsion preparation through the completion of tabular grain growth require only the substitution of the selected peptizer for conventional gelatino-peptizers. The following high bromide {111} tabular grain emulsion precipitation procedures, here incorporated by reference, are specifically contemplated to be useful in the practice of the invention, subject to the selected peptizer modifications discussed above:

- Daubendiek et al U.S. Pat. No. 4,414,310;
- Abbott et al U.S. Pat. No. 4,425,426;
- Wilgus et al U.S. Pat. No. 4,434,226;
- Maskasky U.S. Pat. No. 4,435,501;
- Kofron et al U.S. Pat. No. 4,439,520;
- Solberg et al U.S. Pat. No. 4,433,048;
- Evans et al U.S. Pat. No. 4,504,570;
- Yamada et al U.S. Pat. No. 4,647,528;
- Daubendiek et al U.S. Pat. No. 4,672,027;
- Daubendiek et al U.S. Pat. No. 4,693,964;
- Sugimoto et al U.S. Pat. No. 4,665,012;
- Daubendiek et al U.S. Pat. No. 4,672,027;
- Yamada et al U.S. Pat. No. 4,679,745;
- Daubendiek et al U.S. Pat. No. 4,693,964;
- Maskasky U.S. Pat. No. 4,713,320;
- Nottorf U.S. Pat. No. 4,722,886;
- Sugimoto U.S. Pat. No. 4,755,456;
- Goda U.S. Pat. No. 4,775,617;
- Saitou et al U.S. Pat. No. 4,797,354;
- Ellis U.S. Pat. No. 4,801,522;
- Ikeda et al U.S. Pat. No. 4,806,461;
- Ohashi et al U.S. Pat. No. 4,835,095;
- Makino et al U.S. Pat. No. 4,835,322;
- Daubendiek et al U.S. Pat. No. 4,914,014;
- Aida et al U.S. Pat. No. 4,962,015;
- Ikeda et al U.S. Pat. No. 4,985,350;
- Pigglin et al U.S. Pat. No. 5,061,609;
- Pigglin et al U.S. Pat. No. 5,061,616;
- Tsaur et al U.S. Pat. No. 5,147,771;
- Tsaur et al U.S. Pat. No. 5,147,772;
- Tsaur et al U.S. Pat. No. 5,147,773;
- Tsaur et al U.S. Pat. No. 5,171,659;
- Tsaur et al U.S. Pat. No. 5,210,013;
- Antoniades et al U.S. Pat. No. 5,250,403;
- Kim et al U.S. Pat. No. 5,272,048;
- Delton U.S. Pat. No. 5,310,644;
- Chang et al U.S. Pat. No. 5,314,793;
- Sutton et al U.S. Pat. No. 5,334,469;
- Black et al U.S. Pat. No. 5,334,495;
- Chaffee et al U.S. Pat. No. 5,358,840; and
- Delton U.S. Pat. No. 5,372,927.

The high bromide {111} tabular grain emulsions that are formed preferably contain at least 70 (optimally at least 90)

mole percent bromide, based on silver. Silver bromide, silver iodobromide, silver chlorobromide, silver iodochlorobromide, and silver chloroiodobromide tabular grain emulsions are specifically contemplated. Although silver chloride and silver bromide form tabular grains in all proportions, chloride is preferably present in concentrations of 30 mole percent, based on silver, or less. Iodide can be present in the tabular grains up to its solubility limit under the conditions selected for tabular grain precipitation. Under ordinary conditions of precipitation silver iodide can be incorporated into the tabular grains in concentrations ranging up to about 40 mole percent, based on silver. It is generally preferred that the iodide concentration be less than 20 mole percent, based on silver. Typically the iodide concentration is less than 10 mole percent, based on silver. To facilitate rapid processing, such as commonly practiced in radiography, it is preferred that the iodide concentration be limited to less than 4 mole percent, based on silver. Significant photographic advantages can be realized with iodide concentrations as low as 0.5 mole percent, based on silver, with an iodide concentration of at least 1 mole percent, based on silver, being preferred.

The high bromide {111} tabular grain emulsions can exhibit mean grain ECD's of any conventional value, ranging up to 10  $\mu\text{m}$ , which is generally accepted as the maximum mean grain size compatible with photographic utility. In practice, the tabular grain emulsions of the invention typically exhibit a mean ECD in the range of from about 0.2 to 7.0  $\mu\text{m}$ . Tabular grain thicknesses typically range from about 0.03  $\mu\text{m}$  to 0.3  $\mu\text{m}$ . For blue recording somewhat thicker grains, up to about 0.5  $\mu\text{m}$ , can be employed. For minus blue (red and/or green) recording, thin (<0.2  $\mu\text{m}$ ) tabular grains are preferred.

The advantages that tabular grains impart to emulsions generally increases as the average aspect ratio or tabularity of the tabular grain emulsions increases. Both aspect ratio (ECD/t) and tabularity (ECD/t<sup>2</sup>, where ECD and t are measured in  $\mu\text{m}$ ) increase as average tabular grain thickness decreases. Therefore it is generally sought to minimize the thicknesses of the tabular grains to the extent possible for the photographic application. Absent specific application prohibitions, it is generally preferred that the tabular grains having a thickness of less than 0.3  $\mu\text{m}$  (preferably less than 0.2  $\mu\text{m}$  and optimally less than 0.07  $\mu\text{m}$ ) and accounting for greater than 50 percent (preferably at least 70 percent and optimally at least 90 percent) of total grain projected area exhibit an average aspect ratio of greater than 5 and most preferably greater than 8. Tabular grain average aspect ratios can range up to 100, 200 or higher, but are typically in the range of from about 12 to 80. Tabularities of >25 are generally preferred.

High bromide {111} tabular grain emulsions precipitated in the presence of a cationic starch are disclosed in the following patents, the disclosures of which are here incorporated by reference: Maskasky U.S. Pat. Nos. 5,604,085, 5,620,840, 5,667,955, 5,691,131, and 5,733,718.

Conventional dopants can be incorporated into the tabular grains during their precipitation, as illustrated by the patents cited above and *Research Disclosure*, Item 38957, cited above, Section I. Emulsion grains and their preparation, D. Grain modifying conditions and adjustments, paragraphs (3), (4) and (5). It is specifically contemplated to incorporate shallow electron trapping (SET) site providing dopants in the tabular grains, further disclosed in *Research Disclosure*, Vol. 367, November 1994, Item 36736, and Olm et al U.S. Pat. No. 5,576,171, here incorporated by reference.

It is also recognized that silver salts can be epitaxially grown onto the tabular grains during the precipitation pro-

cess. Epitaxial deposition onto the edges and/or corners of tabular grains is specifically taught by Maskasky U.S. Pat. No. 4,435,501 and Daubendiek et al U.S. Pat. Nos. 5,573,902 and 5,576,168, here incorporated by reference.

Although epitaxy onto the host tabular grains can itself act as a sensitizer, the emulsions of the invention show sensitivity enhancements with or without epitaxy when chemically sensitized employing one or a combination of noble metal, middle chalcogen (sulfur, selenium and/or tellurium) and reduction chemical sensitization techniques. Conventional chemical sensitizations by these techniques are summarized in *Research Disclosure*, Item 38957, cited above, Section IV. Chemical sensitizations. It is preferred to employ at least one of noble metal (typically gold) and middle chalcogen (typically sulfur) and, most preferably, a combination of both in preparing the emulsions of the invention for photographic use. The use of a cationic starch peptizer allows distinct advantages relating to chemical sensitization to be realized. Under comparable levels of chemical sensitization higher photographic speeds can be realized using cationic starch peptizers. When comparable photographic speeds are sought, a cationic starch peptizer in the absence of gelatin allows lower levels of chemical sensitizers to be employed and results in better incubation keeping. When chemical sensitizer levels remain unchanged, speeds equal to those obtained using gelatino-peptizers can be achieved at lower precipitation and/or sensitization temperatures, thereby avoiding unwanted grain ripening.

Between emulsion precipitation and chemical sensitization, the step that is preferably completed before any gelatin or gelatin derivative is added to the emulsion, it is conventional practice to wash the emulsions to remove soluble reaction by-products (e.g., alkali and/or alkaline earth cations and nitrate anions). If desired, emulsion washing can be combined with emulsion precipitation, using ultrafiltration during precipitation as taught by Mignot U.S. Pat. No. 4,334,012. Alternatively emulsion washing by diafiltration after precipitation and before chemical sensitization can be undertaken with a semipermeable membrane as illustrated by *Research Disclosure*, Vol. 102, October 1972, Item 10208, Hagemeyer et al *Research Disclosure*, Vol. 131, March 1975, Item 13122, Bonnet *Research Disclosure*, Vol. 135, July 1975, Item 13577, Berg et al German OLS 2,436,461 and Bolton U.S. Pat. No. 2,495,918, or by employing an ion-exchange resin, as illustrated by Maley U.S. Pat. No. 3,782,953 and Noble U.S. Pat. No. 2,827,428. In washing by these techniques there is no possibility of removing the selected peptizers, since ion removal is inherently limited to removing much lower molecular weight solute ions.

A specifically preferred approach to chemical sensitization employs a combination of sulfur containing ripening agents in combination with middle chalcogen (typically sulfur) and noble metal (typically gold) chemical sensitizers. Contemplated sulfur containing ripening agents include thioethers, such as the thioethers illustrated by McBride U.S. Pat. No. 3,271,157, Jones U.S. Pat. No. 3,574,628 and Rosencrantz et al U.S. Pat. No. 3,737,313. Preferred sulfur containing ripening agents are thiocyanates, illustrated by Nietz et al U.S. Pat. No. 2,222,264, Lowe et al U.S. Pat. No. 2,448,534 and Illingsworth U.S. Pat. No. 3,320,069. A preferred class of middle chalcogen sensitizers are tetra-substituted middle chalcogen ureas of the type disclosed by Herz et al U.S. Pat. Nos. 4,749,646 and 4,810,626, the disclosures of which are here incorporated by reference. Preferred compounds include those represented by the formula:



wherein

X is sulfur, selenium or tellurium;

each of  $R_1$ ,  $R_2$ ,  $R_3$  and  $R_4$  can independently represent an alkylene, cycloalkylene, alkarylene, aralkylene or heterocyclic arylene group or, taken together with the nitrogen atom to which they are attached,  $R_1$  and  $R_2$  or  $R_3$  and  $R_4$  complete a 5 to 7 member heterocyclic ring; and

each of  $A_1, A_2, A_3$  and  $A_4$  can independently represent hydrogen or a radical comprising an acidic group, with the proviso that at least one  $A_1R_1$  to  $A_4R_4$  contains an acidic group bonded to the urea nitrogen through a carbon chain containing from 1 to 6 carbon atoms.

X is preferably sulfur and  $A_1R_1$  to  $A_4R_4$  are preferably methyl or carboxymethyl, where the carboxy group can be in the acid or salt form. A specifically preferred tetra substituted thiourea sensitizer is 1,3-dicarboxymethyl-1,3-dimethylthiourea.

Preferred gold sensitizers are the gold(I) compounds disclosed by Deaton U.S. Pat. No. 5,049,485, the disclosure of which is here incorporated by reference. These compounds include those represented by the formula:



wherein

L is a mesoionic compound;

X is an anion; and

$L^1$  is a Lewis acid donor.

In another preferred form of the invention it is contemplated to employ alone or in combination with sulfur sensitizers, such as those of formula m, and/or gold sensitizers, such as those of formula IV, reduction sensitizers which are the 2-[N-(2-alkynyl)amino]-meta-chalcoazoles disclosed by Lok et al U.S. Pat. Nos. 4,378,426 and 4,451,557, the disclosures of which are here incorporated by reference.

Preferred 2-[N-(2-alkynyl)amino]-meta-chalcoazoles can be represented by the formula:



where

X=O, S, Se;

$R_1$ =(Va) hydrogen or (Vb) alkyl or substituted alkyl or aryl or substituted aryl; and

$Y_1$  and  $Y_2$  individually represent hydrogen, alkyl groups or an aromatic nucleus or together represent the atoms necessary to complete an aromatic or alicyclic ring containing atoms selected from among carbon, oxygen, selenium, and nitrogen atoms.

The formula V compounds are generally effective (with the Vb form giving very large speed gains and exceptional latent image stability) when present during the heating step (finish) that results in chemical sensitization.

The fragmentable electron donating sensitizer provides additional speed when used in place of one, some or all conventional chemical sensitizers or in combination with these sensitizers. It is common practice in chemically sensitizing gelatio-peptized emulsions to hold the emulsions for a period of time at an elevated temperature to effect chemical sensitization. The FED sensitizer can be added before heating when the sensitizer is sufficiently stable to withstand the elevated temperature without fragmenting. However, where a heating step is contemplated to effect a conventional chemical sensitization, it is preferred to add the FED sensitizer at the conclusion of the heating step. One of the significant advantages of this invention is that the oxidized cationic starch peptized emulsions can be efficiently chemically sensitized with conventional sensitizers, such as those of formulae (III), (IV) and (V) above, at lower temperatures. For example, chemical sensitization can be achieved at temperatures lower than those required for the sensitization of corresponding gelatino-peptized emulsions. It is possible to achieve chemical sensitization of oxidized cationic starch peptized tabular grain emulsions by heating to temperatures of <40° C. Thus, the FED sensitizer can be added before, during or after addition of any other, conventional chemical sensitizers.

Fragmentable electron donating (FED) sensitizers of the types disclosed by Farid et al U.S. Pat. Nos. 5,747,235 and 30 5,7547,236; in Lenhard et al U.S. Ser. No. 08/739,911, filed Oct. 30, 1996; and in Gould et al U.S. Ser. No. 09/118,536, Farid et al U.S. Ser. No. 09/118,552, and Adin et al U.S. Ser. No. 09/118,714, each filed June 25, 1998; the disclosures of 35 which are here incorporated by reference, are specifically contemplated for use in the practice of this invention.

These FED sensitizers satisfy the formula  $X—Y'$ ,  $X—Y'$  forming the entire sensitizer or a moiety  $—X—Y'$  of the sensitizer, wherein

40 X is an electron donating compound moiety;

Y' is a proton or a leaving group Y'; and wherein:

- (1) X—Y' has an oxidation potential between 0 and about 1.4 V; and
- (2) the oxidized form of X—Y' undergoes a bond cleavage reaction to give the radical X• and the leaving fragment Y'; and, optionally,
- (3) the radical X• has an oxidation potential  $\leq -0.7$  V (that is, equal to or more negative than about  $-0.7$  V).

50 In embodiments of the invention wherein Y' is a proton, a base,  $B^-$ , is covalently linked directly or indirectly to X

Compounds wherein X—Y' meets criteria (1) and (2) but not (3) are capable of donating one electron and are referred

not (3) are capable of donating one electron and are referred to herein as fragmentable one-electron donating compounds. Compounds which meet all three criteria are capable of donating two electrons and are referred to herein as fragmentable two-electron donating compounds.

60 In this patent application, oxidation potentials are reported as "V" which represents volts versus a saturated calomel reference electrode.

In embodiments of the invention in which Y' is Y, the following represents the reactions that are believed to take place when X—Y undergoes oxidation and fragmentation to produce a radical X•, which in a preferred embodiment undergoes further oxidation.



Electron elimination from compound X—Y occurs when the oxidation potential of X—Y is equal to or more negative than 1.4 volts. Electron elimination from the free radical X• occurs when X• exhibits an oxidation potential equal to or more negative than -0.7 volt.

The structural features of X—Y are defined by the characteristics of the two parts, namely the fragment X and the fragment Y. The structural features of the fragment X determine the oxidation potential of the X—Y molecule and that of the radical X•, whereas both the X and Y fragments affect the fragmentation rate of the oxidized molecule X—Y•.

In embodiments of the invention in which Y' is H, the following represents the reactions believed to take place when the compound X—H undergoes oxidation and deprotonation to the base, B<sup>-</sup>, to produce a radical X•, which in a preferred embodiment undergoes further oxidation.



Preferred X groups are of the general formula:

(VI)



(VII)



(VIII)



(IX)



The symbol "R" (that is R without a subscript) is used in all structural formulae in this patent application to represent a hydrogen atom or an unsubstituted or substituted alkyl group.

In structure (VI):

m=0, 1;

Z=O, S, Se, Te;

Ar=aryl group (e.g., phenyl, naphthyl, phenanthryl, anthryl); or heterocyclic group (e.g., pyridine, indole, benzimidazole, thiazole, benzothiazole, thiadiazole, etc.);

R<sub>1</sub>=R, carboxyl, amide, sulfonamide, halogen, NR<sub>2</sub>, (OH)<sub>n</sub>, (OR)<sub>n</sub>, or (SR)<sub>n</sub>;

R'=alkyl or substituted alkyl;

n=1-3;

R<sub>2</sub>=R, Ar';

R<sub>3</sub>=R, Ar';

R<sub>2</sub> and R<sub>3</sub> together can form 5- to 8-membered ring;

R<sub>2</sub> and Ar' can be linked to form 5- to 8-membered ring;

R<sub>3</sub> and Ar' can be linked to form 5- to 8-membered ring;

Ar'=aryl group such as phenyl, substituted phenyl, or heterocyclic group (e.g., pyridine, benzothiazole, etc.)

R=a hydrogen atom or an unsubstituted or substituted alkyl group.

In structure (VII):

Ar=aryl group (e.g., phenyl, naphthyl, phenanthryl); or heterocyclic group (e.g., pyridine, benzothiazole, etc.);

R<sub>4</sub>=a substituent having a Hammett sigma value of -1 to +1, preferably -0.7 to +0.7, e.g., R, OR, SR, halogen, CHO, C(O)R, COOR, CONR<sub>2</sub>, SO<sub>3</sub>R, SO<sub>2</sub>NR<sub>2</sub>, SO<sub>2</sub>R, SOR, C(S)R, etc.;

R<sub>5</sub>=R, Ar'

R<sub>6</sub> and R<sub>7</sub>=R, Ar'

R<sub>5</sub> and Ar' can be linked to form 5- to 8-membered ring;

R<sub>6</sub> and Ar' can be linked to form 5- to 8-membered ring (in which case, R<sub>6</sub> can be a hetero atom);

R<sub>5</sub> and R<sub>6</sub> can be linked to form 5- to 8-membered ring;

R<sub>6</sub> and R<sub>7</sub> can be linked to form 5- to 8-membered ring;

Ar'=aryl group such as phenyl, substituted phenyl, heterocyclic group;

R=hydrogen atom or an unsubstituted or substituted alkyl group.

A discussion on Hammett sigma values can be found in C.

Hansch and R. W. Taft *Chem. Rev.* Vol 91, (1991) p 165, the disclosure of which is incorporated herein by reference.

In structure (VIII):

W=O, S, Se;

Ar=aryl group (e.g., phenyl, naphthyl, phenanthryl, anthryl); or heterocyclic group (e.g., indole, benzimidazole, etc.);

R<sub>8</sub>=R, carboxyl, NR<sub>2</sub>, (OR)<sub>n</sub>, or (SR)<sub>n</sub> (n=1-3);

R<sub>9</sub> and R<sub>10</sub>=R, Ar';

R<sub>9</sub> and Ar' can be linked to form 5- to 8-membered ring;

Ar'=aryl group such as phenyl substituted phenyl or heterocyclic group;

R=a hydrogen atom or an unsubstituted or substituted alkyl group.

In structure (IX):

"ring" represents a substituted or unsubstituted 5-, 6- or 7-membered unsaturated ring, preferably a heterocyclic ring.

The following are illustrative examples of the group X of the general structure VI:



-continued



In the structures of this patent application a designation such as —OR(NR<sub>2</sub>) indicates that either —OR or —NR<sub>2</sub> can be present.

The following are illustrative examples of the group X of general structure VII:



**19**

-continued



$Z_1$ =a covalent bond, S, O, Se, NR, CR<sub>2</sub>, CR=CR, or CH<sub>2</sub>CH<sub>2</sub>. 45



$Z_2$ =S, O, Se, NR, CR<sub>2</sub>, CR=CR, R<sub>13</sub>, =alkyl, substituted alkyl or aryl, and R<sub>14</sub>=H, alkyl substituted alkyl or aryl. 55

The following are illustrative examples of the group X of the general structure VIII:

**20**

-continued

5



10



15



20

The following are illustrative examples of the group X of the general structure IX:

25



30



35



40

$Z_3$ =O, S, Se, NR

R<sub>15</sub>=R, OR, NR<sub>2</sub>

R<sub>16</sub>=alkyl, substituted alkyl

Preferred Y' groups are:

(1) X', where X' is an X group as defined in structures I-IV and may be the same as or different from the X group to which it is attached

(2)



(3)



55

60

65

where M=Si, Sn or Ge; and R'=alkyl or substituted alkyl



where Ar''=aryl or substituted aryl



In preferred embodiments of this invention Y' is —H, —COO<sup>-</sup> or —Si(R')<sub>3</sub> or —X'. Particularly preferred Y' groups are —H, —COO<sup>-</sup> or —Si(R')<sub>3</sub>. In embodiments of the invention in which Y' is a proton, a base, B<sup>-</sup>, is covalently linked directly or indirectly to X. The base is preferably the conjugate base of an acid of pKa between about 1 and about 8, preferably about 2 to about 7. Collections of pKa values are available (see, for example: *Dissociation Constants of Organic Bases in Aqueous Solution*, D. D. Peril (Butterworths, London, 1965); *CRC Handbook of Chemistry and Physics*, 77th ed, D. R. Lide (CRC Press, Boca Raton, Fla., 1996)). Examples of useful bases are included in Table I.

TABLE I

| pKa's in water of the conjugate acids of some useful bases           |      |
|----------------------------------------------------------------------|------|
| CH <sub>3</sub> —CO <sub>2</sub> <sup>-</sup>                        | 4.76 |
| C <sub>2</sub> H <sub>5</sub> —CO <sub>2</sub> <sup>-</sup>          | 4.87 |
| (CH <sub>3</sub> ) <sub>2</sub> CH—CO <sub>2</sub> <sup>-</sup>      | 4.84 |
| (CH <sub>3</sub> ) <sub>3</sub> C—CO <sub>2</sub> <sup>-</sup>       | 5.03 |
| HO—CH <sub>2</sub> —CO <sub>2</sub> <sup>-</sup>                     | 3.83 |
|                                                                      | 3.48 |
| CH <sub>3</sub> —CO—NH—CH <sub>2</sub> —CO <sub>2</sub> <sup>-</sup> | 3.67 |
|                                                                      | 4.19 |
|                                                                      | 4.96 |
| CH <sub>3</sub> —COS <sup>-</sup>                                    | 3.33 |
|                                                                      | 3.73 |
|                                                                      | 4.88 |

TABLE I-continued

| pKa's in water of the conjugate acids of some useful bases |      |
|------------------------------------------------------------|------|
| 5                                                          | 4.01 |
|                                                            |      |
| 10                                                         | 4.7  |
|                                                            |      |
| (5)                                                        |      |
| 15                                                         |      |
|                                                            | 4.65 |
|                                                            | 6.61 |
| 20                                                         |      |
| 25                                                         |      |
|                                                            | 5.25 |
| 30                                                         |      |
| 35                                                         |      |
|                                                            | 6.15 |
| 40                                                         |      |
|                                                            | 2.44 |
| 45                                                         |      |
|                                                            | 5.53 |

50 Preferably the base, B<sup>-</sup> is a carboxylate, sulfate or amine oxide.

In some embodiments of the invention, the fragmentable electron donating sensitizer contains a light absorbing group, Z, which is attached directly or indirectly to X, directly or indirectly attached to X, or a chromophore forming group, Q, which is attached to X. Such fragmentable electron donating sensitizers are preferably of the following formulae:

Z—(L—X—Y')<sub>k</sub>  
 A—(L—X—Y')<sub>k</sub>  
 (A—L)<sub>k</sub>—X—Y'  
 Q—X—Y'  
 A—(X—Y')<sub>k</sub>  
 (A)<sub>k</sub>—X—Y'  
 Z—(X—Y')<sub>k</sub> or  
 (Z)<sub>k</sub>—X—Y'  
 Z is a light absorbing group;

23

k is 1 or 2;

A is a silver halide adsorptive group that contains at least one atom of N, S, P, Se, or Te that promotes adsorption to silver halide;

L represents a linking group containing at least one C, 5 N, S, P or O atom; and

Q represents the atoms necessary to form a chromophore comprising an amidinium-ion, a carboxyl-

24

ion or dipolar-amidic chromophoric system when conjugated with X—Y'.

Z is a light absorbing group including, for example, cyanine dyes, complex cyanine dyes, merocyanine dyes, complex merocyanine dyes, homopolar cyanine dyes, styryl dyes, oxonol dyes, hemioxonol dyes, and hemicyanine dyes.

Preferred Z groups are derived from the following dyes:



**25**

-continued

**26**

Dye 5



Dye 6



Dye 7



Dye 8



The linking group L may be attached to the dye at one (or more) of the heteroatoms, at one (or more) of the aromatic or heterocyclic rings, or at one (or more) of the atoms of the polymethine chain, at one (or more) of the hetero atoms, at one (or more) of the aromatic or heterocyclic rings, or at one (or more) of the atoms of the polymethine chain. For simplicity, and because of the multiple possible attachment sites, the attachment of the L group is not specifically indicated in the generic structures.

The silver halide adsorptive group A is preferably a silver-ion ligand moiety or a cationic surfactant moiety. In preferred embodiments, A is selected from the group consisting of: i) sulfur acids and their Se and Te analogs, ii) nitrogen acids, iii) thioethers and their Se and Te analogs, iv) phosphines, v) thionamides, selenamides, and telluramides, and vi) carbon acids.

Illustrative A groups include:



27

-continued



The point of attachment of the linking group L to the silver halide adsorptive group A will vary depending on the structure of the adsorptive group, and may be at one (or more) of the heteroatoms, at one (or more) of the aromatic or heterocyclic rings.

The linkage group represented by L which connects the light absorbing group to the fragmentable electron donating group XY by a covalent bond is preferably an organic linking group containing at least one C, N, S, or O atom. It is also desired that the linking group not be completely aromatic or unsaturated, so that a pi-conjugation system cannot exist between the Z and XY moieties. Preferred examples of the linkage group include, an alkylene group, an arylene group, —O—, —S—, —C=O, —SO<sub>2</sub>—, —NH—, —P=O, and —N=. Each of these linking components can be optionally substituted and can be used alone or in combination. Examples of preferred combinations of these groups are:



-continued



25 where  $c=1-30$ , and  $d=1-10$

The length of the linkage group can be limited to a single atom or can be much longer, for instance up to 30 atoms in length. A preferred length is from about 2 to 20 atoms, and most preferred is 3 to 10 atoms. Some preferred examples of L can be represented by the general formulae indicated below:



50 e and f=1–30, with the proviso that  $e+f \leq 30$

Q represents the atoms necessary to form a chromophore comprising an amidinium-ion, a carboxyl-ion or dipolar-amidic chromophoric system when conjugated with X—Y'. Preferably the chromophoric system is of the type generally found in cyanine, complex cyanine, hemicyanine, merocyanine, and complex merocyanine dyes as described in F. M. Hamer, *The Cyanine Dyes and Related Compounds* (Interscience Publishers, N.Y., 1964).

60 Illustrative Q groups include:



**29**

-continued

**30**

-continued



5

10

15

20

wherein:

25

$X_2$  is O, S, N, or  $C(R_{19})_2$ , where  $R_{19}$  is substituted or unsubstituted alkyl.

each  $R_{17}$  is independently a hydrogen atom, a halogen atom, a substituted or unsubstituted alkyl group, or substituted or unsubstituted aryl group;

$a$  is an integer of 1-4; and

$R_{18}$  is substituted or unsubstituted alkyl, or substituted or unsubstituted aryl.

Illustrative fragmentable electron donating sensitizers include:

40



FED 1



FED 2





-continued

FED 9



FED 10



FED 11



FED 12



FED 13



FED 14



-continued

FED 15



FED 16



FED 17



FED 18



-continued

FED 19



FED 20



FED 21



FED 22



In a preferred form of the invention one or more spectral sensitizing dyes are adsorbed to the surfaces of the high bromide {111} tabular grains. In one specifically preferred form of the invention, the FED sensitizer includes a dye chromophore, providing the photon capture capability of a spectral sensitizing dye and the additional electron injection capability of a FED sensitizer. This allows a dye chromophore containing FED sensitizer to be substituted for a conventional spectral sensitizing dye. Spectral sensitizing dyes of conventional types and in conventional amounts are contemplated for use with the FED sensitizers. A FED sensitizer containing a chromophore, when employed in combination with one or more conventional spectral sensitizing dyes, can be chosen to absorb light in the same spectral region or a different spectral region than the conventional spectral sensitizing dye. As previously noted, a summary of spectral sensitizing dyes is provided by *Research Disclosure*, Item 38957, V. Spectral sensitization and desensitization, A. Sensitizing Dyes, cited above. Typically spectral sensitizing dyes are adsorbed to the surfaces of the grains after chemical sensitization, but advantages for dye addition to high bromide {111} tabular grains prior to or during chemical sensitization have long been recognized, as is illustrated by Kofron et al U.S. Pat. No. 4,439,520. The FED

45 sensitizer can be added to the emulsion prior to, during or following spectral sensitization.

The FED sensitizer can be incorporated in the emulsion by the conventional techniques for dispersing spectral sensitizing dyes. That is, the FED sensitizer can be added directly to the emulsion or added after being dissolved in a 50 solvent, such as water, methanol or ethanol, or a mixture of solvents (e.g., an aqueous alcoholic solution). The FED sensitizers may also be added from solutions containing base and/or surfactants. The FED sensitizers may also be incorporated in aqueous slurries or peptizer dispersions.

55 FED sensitizers are added to the emulsions of the invention to allow intimate contact with the high bromide {111} tabular grains. In preferred forms the FED sensitizers are adsorbed to the grain surfaces. FED sensitizer concentrations in the emulsions of the invention can range from as low as  $1 \times 10^{-8}$  mole per silver mole up to 0.1 mole per silver mole. A preferred concentration range is about  $5 \times 10^{-7}$  to 0.05 mole per silver mole. It is appreciated that the more active forms of the FED sensitizer (e.g., those capable of injecting a higher number of electrons per molecule) can be employed in lower concentrations while achieving the same 60 advantageous effects as less active forms. Although it is preferred that the FED sensitizer be added to the emulsion

of the invention before, during or immediately following the addition of other conventional incorporated sensitizers, increases in emulsion sensitivity have been observed even when FED sensitizer addition has been delayed until after the emulsion has been coated.

In addition to high bromide {111} tabular grains, cationic starch peptizer, and FED sensitizer, usually in combination with conventional chemical and/or spectral sensitizers, the emulsions of the invention additionally preferably include one or more conventional antifoggants and stabilizers. A summary of conventional antifoggants and stabilizers is contained in *Research Disclosure*, Item 38957, VII. Antifoggants and stabilizers.

It has been observed that employing a FED sensitizer in combination with a cationic starch peptizer results in somewhat higher minimum densities than when a gelatinopeptizer is substituted, even when conventional antifoggants and stabilizers are present in the emulsion. It has been discovered that this incremental increase in minimum density can be reduced or eliminated by treating the emulsion with an oxidizing agent during or subsequent to grain precipitation. Preferred oxidizing agents are those that in their reduced form have little or no impact on the performance properties of the emulsions in which they are incorporated. Strong oxidizing agents noted above to be useful in oxidizing cationic starch, such as hypochlorite ( $\text{ClO}^-$ ) or periodate ( $\text{IO}_4^-$ ), are specifically contemplated. Specifically preferred oxidizing agents are halogen—e.g., bromine ( $\text{Br}_2$ ) or iodine ( $\text{I}_2$ ). When bromine or iodine is used as an oxidizing agent, the bromine or iodine is reduced to  $\text{Br}^-$  or  $\text{I}^-$ . These halide ions can remain with other excess halide ions in the dispersing medium of the emulsion or be incorporated within the grains without adversely influencing photographic performance. Any level of oxidizing agent can be utilized that is effective in reducing minimum density. Concentrations of oxidizing agent added to the emulsion as low as about  $1 \times 10^{-6}$  mole per Ag mole are contemplated. Since very low levels of  $\text{Ag}^\circ$  are responsible for increases in minimum density, no useful purpose is served by employing oxidizing agent concentrations of greater than 0.1 mole per Ag mole. A specifically preferred oxidizing agent range is from  $1 \times 10^{-4}$  to  $1 \times 10^{-2}$  mole per Ag mole. The silver basis is the total silver at the conclusion of precipitation of the high bromide {111} tabular grain emulsion, regardless of whether the oxidizing agent is added during or after precipitation.

Element I illustrates a photographic element according to the invention having its construction reduced to essential features.

---

Emulsion Layer Unit  
Support  
Element I

---

The Emulsion Layer Unit can consist of a single high bromide {111} tabular grain emulsion according to the invention containing FED sensitizer and a cationic starch peptizer as described above. The cationic starch peptizer added during emulsion precipitation typically forms only a small portion of the total vehicle of the emulsion layer. Additional cationic starch of the type used as a peptizer can be added to act as a binder. However, it is preferred to employ as binders other conventional hydrophilic colloid binders, particularly gelatin and gelatin derivatives. Maskasky U.S. Pat. No. 5,726,008, here incorporated by reference, describes a vehicle that can be chill set containing

at least 45 percent by gelatin and at least 20 percent of a water dispersible starch. In addition to peptizer and binder, the vehicle is reacted with a hardener to increase its physical integrity as a coating and other addenda, such as latices, are

5 also commonly incorporated. Conventional components which can be included within the vehicle of the emulsion layer summarized in *Research Disclosure*, Item 38957, II. Vehicles, vehicle extenders, vehicle-like addenda and vehicle related addenda and IX. Coating physical property 10 modifying addenda—e.g., coating aids (such as surfactants), plasticizers and lubricants, matting agents and antistats are common vehicle components, conventional choices being illustrated by *Research Disclosure*, Item 38957, IX. Coating physical property modifying addenda.

15 Although individual organic vehicles differ somewhat in their refractive indices, all have refractive indices nearer to gelatin (1.54) than to silver halide (2.0 to 2.2, depending on the halide). Virtually all organic materials have refractive indices less than  $\pm 10\%$  of the refractive index of gelatin.

20 To add an additional increment of speed to the performance of the emulsion layer, it is contemplated to add light scattering particles to the emulsion layer. Light scattering characteristics are a function of (a) the refractive index of the particle material, (b) the size of the particle, and (c) the 25 shape of the particle.

The particles have an aspect ratio of less than 1.5. The 30 purpose of limiting the particle aspect ratio is to assure that the particles are randomly oriented in the emulsion layer. Thus, non-oriented light scatter is achieved as opposed to 35 specular reflection, as is commonly observed to occur from tabular silver halide grains due to their orientation of major faces parallel to the support surface. In a preferred form the particles are isotropic—that is, they have an aspect ratio of approximately unity.

35 The size of the particles also influences their light scattering capability. Generally maximum light scattering occurs when the wavelength of exposing radiation matches the equivalent spherical diameter of a particle. An equivalent spherical diameter (or ESD) is the diameter of a sphere 40 having a volume equal to that of the particle. It is contemplated to employ particles having mean ESD's in the range of from 0.1 to  $1.0 \mu\text{m}$ . Preferred mean particle ESD's are in the range of from  $\pm 0.2 \mu\text{m}$  of the wavelength of exposing light. For exposures to visible light (400 to 700 nm), 45 preferred mean ESD's of from 0.2 to  $0.8 \mu\text{m}$  (200 to 800 nm).

Ideally all of the particles are sized for efficient light scatter. In practice it is not possible to create populations of fine particles that are identical in size. Preferred particle 50 populations are monodisperse. Monodisperse particles exhibit a coefficient of variation (COV) of less than 20 percent and preferably less than 10 percent, where COV is the 100 times the standard deviation of particle size (ESD) divided by mean particle size. For most efficient particle utilization it is contemplated to employ particle populations in which at least 90% by weight of the particles less than the mean particle size (ESD) are within 40% of the mean particle size while at least 90% by number of the particles greater than the mean particle size are within 40% of the 55 mean particle size.

The materials from which the particles are formed are chosen to exhibit a refractive index that differs significantly from that of the hydrophilic colloid vehicle of the emulsion layer. A minimum particle refractive index of at least 1.9 is 60 preferred at the wavelength of exposing radiation. It is specifically preferred to employ particles that exhibit a refractive index of at least 2.0. Silver bromide has a higher 65

refractive index than silver chloride and hence high (>50 mole percent, based on silver) bromide silver halide particles are preferred over high chloride silver halide particles. Silver iodide exhibits a higher refractive index than either silver chloride or silver bromide. It is specifically contemplated to incorporate minor amounts of silver iodide into particles containing silver chloride and/or bromide to increase their effective refractive index. Zinc oxide, illustrative of a suitable particle material other than silver halide, has a refractive index of 2.0.

In addition to the ability of the particles to scatter light, particle selection also entails consideration of the degree, if any, to which they adversely affect imaging performance of the radiation-sensitive silver halide grains. Materials that have a desensitizing action on the radiation-sensitive silver halide grains are preferably avoided.

Finally, to avoid haziness and/or elevated minimum densities in the emulsion layer following imagewise exposure and processing, it is contemplated to choose particles that can be dissolved for removal from the emulsion layer prior to viewing. For example, Yutzy et al U.K. Specification 760,775 discloses removing zinc oxide particles by treatment of an imagewise exposed and processed emulsion layer with acetic acid under a nitrogen atmosphere to avoid the risk of fog formation. By employing silver halide particles it is possible to remove the particles during the course of conventional color photographic processing without modification.

In a specifically preferred form of the invention the light scattering particles incorporated in the emulsion layer are silver halide particles that can be removed in conventional color negative processing. The following represents a specific reference processing sequence for judging the removal capability of the light scattering particles:

| step    | time  | bath | temperature |
|---------|-------|------|-------------|
| develop | 3'15" | D    | 37.8° C.    |
| bleach  | 4'    | B    | 37.8° C.    |
| wash    | 3'    | W    | 35.5° C.    |
| fix     | 4'    | F    | 37.8° C.    |
| wash    | 3'    | W    | 35.5° C.    |
| rinse   | 1'    | R    | 37.8° C.    |

wherein

'represents minutes;

"represents seconds;

bath D exhibits the following composition:

|                                              |          |
|----------------------------------------------|----------|
| water                                        | 800.0 mL |
| potassium carbonate, anhydrous               | 34.30 g  |
| potassium bicarbonate                        | 2.32 g   |
| sodium sulfite, anhydrous                    | 0.38 g   |
| sodium metabisulfite                         | 2.96 g   |
| potassium iodide                             | 1.20 mg  |
| sodium bromide                               | 1.31 g   |
| diethylenetriaminepentaacetic acid           | 8.43 g   |
| pentasodium salt (40% soln)                  |          |
| hydroxylamine sulfate                        | 2.41 g   |
| N-(4-amino-3-methylphenyl)-N-ethyl-          | 4.52 g   |
| 2-aminoethanol                               |          |
| water to make                                | 1.0 L    |
| pH @ 26.7° C. 10.00 +/- 0.05;                |          |
| bath B represents the following composition: |          |

|                                |          |
|--------------------------------|----------|
| water                          | 500.0 mL |
| 1,3-propylenediamine tetra-    |          |
| acetic acid                    | 37.4 g   |
| 57% ammonium hydroxide         | 70.0 mL  |
| acetic acid                    | 80.0 mL  |
| 2-hydroxy-1,3-propylenediamine | 0.8 g    |

-continued

|   |                            |         |
|---|----------------------------|---------|
| 5 | tetraacetic acid           | 25.0 g  |
|   | ammonium bromide           | 44.85 g |
|   | ferric nitrate nonahydrate | 1.0 L   |
|   | water to make              |         |
|   | pH 4.75;                   |         |

bath F represents the following composition:

|    |                                     |          |
|----|-------------------------------------|----------|
| 10 | water                               | 500.0 mL |
|    | ammonium thiosulfate (58% solution) | 214.0 g  |
|    | (ethylenedinitrilo)tetraacetic acid | 1.29 g   |
|    | disodium salt, dihydrate            |          |
|    | sodium metabisulfite                | 11.0 g   |
|    | sodium hydroxide (50% solution)     | 4.70 g   |
|    | water to make                       | 1.0 L    |
|    | pH at 26.7° C. 6.5 +/- 0.15;        |          |

bath R represents the following composition:

|    |                                                                 |            |
|----|-----------------------------------------------------------------|------------|
| 20 | water                                                           | 900.0 mL   |
|    | 0.5% aqueous p-tertiary-octyl-( $\alpha$ -phenoxypropyl)alcohol | 3.0 mL     |
|    | water to make                                                   | 1.0 L; and |
|    | bath W represents water.                                        |            |

The above process conforms to the Kodak Flexicolor™ C-41 color negative process.

25 To achieve significant light scattering the particles should account for at least 2 (preferably at least 5) percent by weight of the combined weight of silver halide grains and particles in the emulsion layer. The particle loading of the emulsion layer can range up to 50 (preferably up to 25) percent of the combined weight of the grains and particles.

30 When the particles are themselves silver halide grains, they are preferably regular, non-tabular grains. Regular grains are those that are internally free of stacking faults, such as twin planes or screw dislocations. Commonly the regular grains are cubic, octahedral, or tetrahedahedral. The 35 corners and/or edges of the grains can be rounded by ripening and, in the case of extensive ripening, the grains can appear spherical.

To maximize the light scattering capability of particles it is contemplated to blend them with the radiation-sensitive 40 silver halide grains after the latter have been sensitized. In this way FED sensitizer, spectral sensitizing dye and other addenda intended to increase light capture remain primarily adsorbed to the surfaces of the radiation-sensitive grains while the light scattering properties of the particles remain at or near their maximum capability.

The Support can take the form of any conventional photographic element support. Typically the Support is either transparent (e.g., a transparent film support) or a white reflective support (e.g., a photographic paper support). A 50 listing of photographic element supports is provided in *Research Disclosure*, Item 38957, XV. Supports. In the majority of applications higher imaging speeds have been particularly sought for camera speed or "taking" films that have a transparent support. When the film has a transparent support and forms a negative dye image, the image bearing processed film is most commonly used as an exposure master for creating a viewable positive image in a print element (e.g., color paper). When the film has a transparent support and forms a positive dye image, the image is most 55 commonly viewed directly by projection. Where the dye image in the film is to be retrieved by scanning, a taking film of increased speed can be realized by employing a reflective support. It is specifically contemplated to employ a support that is specularly reflective at the time of imagewise exposure, thereby increasing its imaging speed, but is converted to a transparent form during processing to facilitate conventional uses of taking films. Maskasky et al U.S. Ser.

No. 09/118,172, filed Jul. 17, 1998, titled DYE IMAGE FORMING PHOTOGRAPHIC ELEMENT AND PROCESSING TO PRODUCE A VIEWABLE IMAGE, commonly assigned to discloses employing a transparent film support bearing a silver mirror coating that is capable of removal during photographic processing.

In practice, additional features are usually present in a photographic element construction. Elements IIa and IIb illustrate common photographic element constructions useful for black-and-white imaging or producing a single color dye image.

---

|                        |
|------------------------|
| Protective Overcoat    |
| Emulsion Layer Unit    |
| Antihalation Layer     |
| Support                |
| Magnetic Imaging Layer |
| Element IIa            |
| Protective Overcoat    |
| Emulsion Layer Unit    |
| Support                |
| Pelloid Layer          |
| Magnetic Imaging Layer |
| Element IIb            |

---

The Support can take any of the forms described above—i.e., any conventional form. In Element IIa the Antihalation Layer is interposed between the Support and the Emulsion Layer Unit. When the Support is transparent, the Antihalation Layer can be moved to be back side of the Support, as shown in Element IIb, and becomes the Pelloid Layer. The Pelloid Layer also acts as both an antihalation layer and an anti-curl layer. The Antihalation Layer and Pelloid Layer each contain one or more dyes capable of being rendered colorless (i.e., discharged) during photographic processing. Dyes of this type are listed in *Research Disclosure*, Item 38957, VII. Absorbing and scattering materials, B. Absorbing materials and C. Discharge.

The Protective Overcoat is provided to protect the Emulsion Layer Unit. Each of the Antihalation Layer, Pelloid Layer and Protective Overcoat contain a vehicle. The vehicle is comprised of binder, hardener, and selections of the remaining components of the emulsion layer described above. The surface layers, the Pelloid Layer and the Protective Overcoat, are particularly preferred locations for surface modifying addenda, such as lubricants, matting agents and antistats. The Protective Overcoat is also a preferred location for the incorporation of UV stabilizers, a summary disclosure of which is provided in *Research Disclosure*, Vol. 370, February 1995, Item 37038, X. UV Stabilizers.

The Magnetic Imaging Layer is an optional, but preferred layer having as its purpose to store information about the photographic element for use in exposure or subsequent processing. Magnetic imaging layers are illustrated by *Research Disclosure*, Item 38957, XIV. Scan facilitating features and James U.S. Pat. Nos. 5,254,441 and 5,254,449.

Although the Emulsion Layer Unit can consist of a single starch peptized, FED sensitizer containing high bromide {111} tabular grain emulsion (hereinafter referred to as an invention emulsion), it is recognized that the Emulsion Layer Unit can contain a blend of invention emulsions or a blend of one or more invention emulsions and one or more conventional emulsions. It is also common practice to divide emulsion layer units into two or three separate emulsion layers, differing in imaging speed.

By forming the Emulsion Layer Unit of a faster emulsion layer and a slower emulsion layer, with the faster emulsion

layer positioned to first receive exposing radiation (i.e., positioned farther from the support), a higher speed is realized than when the faster and slower emulsions are blended in a single layer. When the slower emulsion layer is positioned to first receive exposing radiation, a higher contrast is realized than when the faster and slower emulsions are blended and coated in a single layer. When three separate emulsions are coated, the third emulsion layer is interposed between the faster and slower emulsions and is chosen to exhibit an intermediate speed. The function of the third emulsion layer is to allow longer exposure latitudes to be realized. Chang and Friday U.S. Pat. Nos. 5,314,793 and 5,360,703, here incorporated by reference, disclose emulsion layer units containing three emulsion layers differing in speed to provide a useful exposure latitude of greater than 1.0 log E.

When one or more other emulsions are employed in combination with the invention emulsion in the Emulsion Layer Unit of Elements I, IIa or IIb, they can be chosen from 20 among conventional negative-working radiation-sensitive silver halide emulsions, such as those described in *Research Disclosure*, Item 38957, I. Emulsion grains and their preparation, with paragraph E. Blends, layers and performance categories, further illustrating emulsion combinations. When one or more conventional emulsions are employed in combination with one or more invention emulsions, the invention emulsions are preferred choices for higher speeds, since they exhibit unexpectedly high speeds. When a conventional emulsion is present in an Emulsion 30 Layer Unit with a invention emulsion, it is preferably also a high (>50 mole percent, based on silver) bromide emulsion, and it is in most instances also a tabular grain emulsion.

Elements I, IIa and IIb can be employed to form a silver image on photographic processing without any further additions to the Emulsion Layer Unit. Reversal dye images can be formed in the photographic elements of the invention without incorporating any dye forming compounds. Techniques for color reversal processing in which dye forming compounds are introduced during reversal processing are 40 disclosed by Mannes et al U.S. Pat. No. 2,52,718, Schwan et al U.S. Pat. No. 2,950,970, and Pilato U.S. Pat. No. 3,547,650. Color reversal dye formation in these types of photographic elements can be achieved using the Kodachrome™ K-14 color reversal process.

To simplify processing, it is usually preferred to incorporate a dye imaging forming compound in the Emulsion Layer Unit when a dye image is desired. The image dye image can, if desired, supplement developed silver in providing a viewable dye. In this arrangement is usually preferred to employ one or a combination of dye image forming compounds capable of forming a neutral density dye image. Thus, Elements I, IIa and IIb can take the form of conventional black-and-white elements (those relying exclusively on developed silver for image density) or so-called chromogenic black-and-white elements (those also relying on neutral density dye for image density). Where a dye image is sought having a specific color, as opposed to a neutral hue, the developed silver is usually removed in processing.

Conventional incorporated dye image providing compounds that can be present in the Emulsion Layer Unit are summarized in *Research Disclosure*, Item 38957, X. Dye image formers and modifiers. Preferred dye image providing compounds are image dye-forming couplers, illustrated in paragraph B. Dye image providing compounds can be 60 incorporated directly into the emulsion layer or, less commonly, are coated in a conventional vehicle containing layer in reactive association with (usually contiguous to) an

emulsion layer. Dye-forming couplers are commonly dispersed in hydrophilic colloid vehicles in high boiling coupler solvents or in latex particles. These and other conventional dispersing techniques are disclosed in paragraph D. Dispersing dyes and dye precursors.

The following is a typical construction of a full color recording photographic element according to the invention—that is, an element capable of recording sufficient image information to allow the image and colors of the photographic subject to be reproduced, either within the color recording photographic element itself or in another color recording photographic element:

|                                            |
|--------------------------------------------|
| Protective Overcoat                        |
| 3 <sup>rd</sup> Color Recording Layer Unit |
| 2 <sup>nd</sup> Interlayer                 |
| 2 <sup>nd</sup> Color Recording Layer Unit |
| 1 <sup>st</sup> Interlayer                 |
| 1 <sup>st</sup> Color Recording Layer Unit |
| Undercoat                                  |
| Transparent Film Support                   |
| Pelloid                                    |
| Magnetic Imaging Layer                     |
| Color Recording Element                    |

The Support and the 1<sup>st</sup>, 2<sup>nd</sup> and 3<sup>rd</sup> Color Recording Layer Units are essential components for all color recording applications. The remaining components are either optional or required only in specific applications. The Protective Overcoat, Transparent Film Support, Pelloid and Magnetic Imaging Layer have been described above and require no further comment.

Each of the Recording Layer Units is an Emulsion Layer Unit constructed of the components described above, except as noted below, that has been chosen to be responsive to one of the blue, green and red portions of the visible spectrum. At least one invention emulsion is present in at least one and preferably each of the Recording Layer Units. Any one of the following layer unit sequences is possible:

|      |                 |
|------|-----------------|
| SQ-1 | B G R  S  ,     |
| SQ-2 | B R G  S  ,     |
| SQ-3 | G R B  S  ,     |
| SQ-4 | R G B  S  ,     |
| SQ-5 | G B R  S  , and |
| SQ-6 | R B G  S        |

where

B=Blue Recording Layer Unit,  
G=Green Recording Layer Unit,  
R=Red Recording Layer Unit, and  
S=Transparent Film Support.

Each of the blue, green and red recording layer units preferably contains a dye image providing compound that produces a dye image of a different hue. When the dye images in the Color Recording Element are intended for direct viewing (e.g., when forming a color slide image or when used as an exposure master for a color print element), the blue, green and red recording layer units are constructed to produce yellow, magenta and cyan dye images, respectively. Preferably the Blue Recording Layer Unit contains a yellow dye-forming coupler, the Green Recording Layer Unit contains a magenta dye-forming coupler, and the Red Recording Layer Unit contains a cyan dye-forming coupler. In addition, conventional image dye modifiers can be incorporated in the Recording Layer Unit, such as those described

in *Research Disclosure*, Item 38957, X. Dye image formers and modifiers, C. Image dye modifiers and D. Hue modifiers/stabilization.

The 1<sup>st</sup> and 2<sup>nd</sup> Interlayers and the Undercoat can contain the same selections of vehicles as described above. The Undercoat can be replaced by the Antihalation Layer described above allowing the Pelloid can be omitted. The 1<sup>st</sup> and 2<sup>nd</sup> Interlayers preferably contain oxidized developing agent scavengers to prevent color developing agent oxidized in one layer unit from migrating to an adjacent layer unit. Typical oxidized developing agent scavengers include balanced (i.e., immobilized) hydroquinone and aminophenol developing agents.

When image information is intended to be read from the photographic elements of the invention by reflection and/or transmission scanning, it is entirely feasible, but no longer of any importance, to form an image that is pleasing to the eye, as in color reversal films, or to form a negative image that can be exposed through to obtain a visually pleasing positive image, as in most color negative films. It is merely necessary that the 1<sup>st</sup>, 2<sup>nd</sup> and 3<sup>rd</sup> Layer Units when exposed and processed contain a retrievable record of the subject, including its color. False color records are just as useful for this purpose as natural color records, and it is, in fact, possible to form three retrievable color records without actually forming three dye images. Color negative films intended solely for scanning do not require masking couplers. Bohan U.S. Pat. No. 5,434,038 discloses a color negative film containing a masking coupler that is equally suited for image retrieval by printing or scanning. Color recording photographic element constructions specifically adapted for the scan retrieval of image information are illustrated by *Research Disclosure*, Item 38957, XIV. Scan facilitating features, Paragraph (1). In addition, the disclosures of the following more recently issued patents of color recording photographic element constructions particularly adapted for scan image retrieval are here incorporated by reference: Sutton et al U.S. Pat. Nos. 5,300,413 and 5,334,469, Sutton U.S. Pat. Nos. 5,314,794 and 5,389,506, Evans et al U.S. Pat. No. 5,389,503, Simons et al U.S. Pat. No. 5,391,443, Simons U.S. Pat. No. 5,418,119 and Gasper et al U.S. Pat. No. 5,420,003.

It has been a long standing practice in the art to modify an edge of color recording film to provide an information record entirely separate from the color image record. For example, edge sound tracks are frequently provided on motion picture films. Modified edge region constructions are illustrated by *Research Disclosure*, Item 38957, XIV. Scan facilitating features, Paragraph (3).

As an alternative to constructing a full color recording photographic element with single blue, green and red recording layer units, it is common practice to provide two or even three layer units for recording in the same region of the spectrum. The most common reason for these constructions is to allow the fastest emulsion for recording in a particular region of the spectrum to receive exposing light prior to transmission through the slower emulsion layers of other layer units. This increases speed and image sharpness. Color recording photographic elements having varied arrangements of layer units, including at least two separate layer units for recording exposure to the same region of the spectrum are illustrated by *Research Disclosure*, Item 38957, XI. Layers and layer arrangements.

The following are illustrative of only a few of the many possible additional layer unit sequences including at least two layer units for recording exposures to the same region of the spectrum:

|       |                                                  |
|-------|--------------------------------------------------|
| SQ-7  | $ B G_f R_f G_s R_s  S  ,$                       |
| SQ-8  | $ B_f G_f R_f B_f G_s R_s  S  ,$                 |
| SQ-9  | $ B G_f R_f G_m R_m G_s R_s  S  ,$               |
| SQ-10 | $ G_f R_f B_f G_s R_s  B_s  S  ,$                |
| SQ-11 | $ G_f R_f B_f G_m R_m B_m G_s R_s B_s  S  ,$ and |
| SQ-12 | $ R_f B G_f R_f G_s R_s  S  $                    |

where

B, G, R and S are as defined above,

f=higher or highest speed of layer units recording in the same region of the spectrum,

m=intermediate speed of layer units recording in the same region of the spectrum,

s=slower or slowest speed of layer units recording in the same region of the spectrum.

In SQ-12 two  $R_f$  layer units are shown. The  $R_f$  layer unit farthest from the support contains a much lower silver halide coating coverage than the remaining  $R_f$  layer unit and is sometimes referred to as a skim coat. Its function is offer a small speed boost to the red record to compensate for the otherwise less favorable for speed and sharpness locations of the red recording layer units as compared to the green recording layer units.

More specific illustrations of full color recording layer units that can be readily modified by the inclusion of one or more invention emulsions are provided by *Research Disclosure*, Item 37038

XIX. Color Negative Example 1

XX. Color Negative Example 2

XXI. Color Reversal Example 1

XXII. Color Reversal Example 2

Full color recording photographic elements are typically employed to record exposures over the full range of the visible spectrum. Occasionally color recording photographic elements are employed to record also exposures in the near ultraviolet and/or near infrared portions of the spectrum. When this is undertaken, an additional layer unit can be provided for this purpose.

Any convenient conventional technique for imagewise exposing a photographic element according to the invention can be employed. Conventional techniques are summarized in *Research Disclosure*, Item 38957, XVI. Exposure.

Exposure (E), measured in lux-seconds, is the product of exposure intensity (I), measured in lux, and time of exposure (ti), measured in seconds:

$$E = (I)(ti)$$

Common photographic applications span light exposures ranging from  $10^{-5}$  to  $10^3$  seconds, and even relatively inexpensive cameras can accommodate exposures ranging from  $10^{-3}$  to  $10^2$  seconds. According to the law of reciprocity, all combinations of varied exposure times and varied exposure intensities that produce the same product (i.e., the same exposure) result in the same image density. In fact, the performance of photographic elements shows varying levels of departure from the law of reciprocity, commonly referred to as reciprocity failure. For example, whereas, according to the law of reciprocity failure a plot of densities versus exposure times (ti), where overall exposure (E) is held constant should result in a curve of invariant density, in practice density variations (reciprocity failure) is observed. It has been observed quite unexpectedly, in comparing otherwise similar starch peptized high bromide {111} tabular grain emulsions with gelatin peptized high bromide {111} tabular grain emulsions, that the starch peptized

emulsions exhibit significantly reduced reciprocity failure (i.e., more closely conform to the law of reciprocity).

Conventional techniques for processing imagewise exposed photographic elements of the invention are contemplated. Typical convenient conventional techniques are illustrated by *Research Disclosure*, Item 38957:

#### XVII. Chemical development systems

- A. Non-specific processing features
- B. Color-specific processing features

#### XIX. Development

- A. Developing Agents
- B. Preservatives
- C. Antifoggants
- D. Sequestering Agents
- E. Other additives

#### XX. Desilvering, washing, rinsing and stabilizing

- A. Bleaching
- B. Fixing
- C. Bleach-Fixing
- D. Washing, rinsing and stabilizing and *Research Disclosure*, Item 37038

#### XXIII. Exposure and processing

- B. Color Film Processing.

Exposure of camera speed color recording photographic elements in limited use and recyclable cameras is specifically contemplated. Limited use camera and incorporated film constructions are the specific subject matter of Item 338957, Section XVI Exposure, cited above, paragraph (2).

Although *Research Disclosure*, Items 36544 and 37038, have been used to provide specific illustrations of conventional photographic element features as well as their exposure and processing, it is recognized that numerous other publications also disclose conventional features, including the following:

James *The Theory of the Photographic Process*, 4th Ed., Macmillan, New York, 1977;

*The Kirk-Othmer Encyclopedia of Chemical Technology*, John Wiley and Sons, New York, 1993;

Nebblette's *Imaging Processes and Materials*, Van Nostrand Reinhold, New York 1988; and

Keller, *Science and Technology of Photography*, VCH, New York, 1993.

#### EXAMPLES

The invention can be better appreciated by reference to the following specific embodiments.

##### Example 1

###### Emulsion S1 (example)

A starch solution was prepared by heating at 85° C. for 45 min a stirred mixture of 8L distilled water and 160 g of an oxidized cationic waxy corn starch. (The starch derivative, STA-LOK® 140 is 100% amylopectin that had been treated to contain quaternary ammonium groups and oxidized with 2 wt % chlorine bleach. It contains 0.31 wt % nitrogen and 0.00 wt % phosphorous. It was obtained from A. E. Staley Manufacturing Co., Decatur, Ill.) After cooling to 40° C., the weight was adjusted to 8.0 kg with distilled water, 26.5 mL of a 2 M NaBr solution was added, then while maintaining the pH at 5.0, 2.0 mL of saturated bromine water (~0.9 mmole) was added dropwise just prior to use.

To a vigorously stirred reaction vessel of the starch solution at 40° C. and maintained at pH 5.0 throughout the emulsion precipitation, a 2.5 M AgNO<sub>3</sub> solution was added

at 200 mL per min for 21 sec. Concurrently, a salt solution of 2.5 M NaBr and 0.4 g/L bromine was added initially at 200 mL per min and then at a rate needed to maintain a pBr of 2.11. Then the addition of the solutions was stopped, 94 mL of the salt solution was added in 1 min and the temperature of the contents of the reaction vessel was increased to 60° C. at a rate of 1.67 ° C. per min. After holding at 60° C. for 10 min, 240 mL of the AgNO<sub>3</sub> solution was added at 10 mL per min for 1 min then its addition rate was accelerated to 19 mL per min in 12 min. The salt solution was concurrently added at a rate needed to maintain a constant pBr of 1.44. The additions were stopped and 40 mL of a buffer solution consisting of 2.94 M sodium acetate and 1.00 M acetic acid was added. Then the addition of the AgNO<sub>3</sub> solution was accelerated from 19 to 54 mL per min in 45 min and then held at this flow rate until a total of 2.4 L of AgNO<sub>3</sub> solution had been added. A solution of 2.5 M NaBr, 0.04 M KI and 0.45 g per L of bromine was concurrently added to maintain a pBr of 1.44. The total making time of the emulsion was ~87 min.

The resulting tabular grain emulsion was washed by ultrafiltration at 40° C. to a pBr of 3.26. Then 27 g of bone gelatin (methionine content ~55 micromole per g gelatin) per mole silver was added.

The {111} tabular grains had an average equivalent circular diameter of 3.8  $\mu$ m, an average thickness of 0.07  $\mu$ m, and an average aspect ratio of 54. The tabular grain population made up 99% of the total projected area of the emulsion grains.

#### Emulsion G1 (control)

To a solution of 10 g low methionine bone gelatin (methionine content <3 micromole per g gelatin), in 7.0 L distilled water and 46 mmole of NaBr at 40° C., pH 5.0 was added 0.10 mL of bromine water. To a vigorously stirred reaction vessel of this gelatin solution at 40° C., maintained at pH 5.0 throughout the precipitation, a 2.5 M AgNO<sub>3</sub> solution was added at 200 mL per min for 21 sec. Concurrently, a salt solution of 2.5 M NaBr and 0.4 g/L bromine was added initially at 200 mL per min and then at a rate needed to maintain a pBr of 2.11. Then the addition of the solutions was stopped, 82 mL of the salt solution was added in 1 min and the temperature of the contents of the reaction vessel was increased to 60° C. at a rate of 1.67° C. per min. Then all but 1.750 kg of the seed emulsion (0.042 mole Ag) was discarded. After the seed emulsion was at 60° C. for a total of 22 min, a solution preheated to 60° C. containing 100 g of oxidized bone gelatin, 1 L distilled water, 15.3 mL of 2 M NaBr and pretreated at 40° C. with 2.0 mL of bromine water was added. Then at 60° C., the AgNO<sub>3</sub> solution was added at 1.0 mL per min for 1 min then accelerated to 25 mL per min in 150 min and held at this flow rate until a total of 2,453 mL of the AgNO<sub>3</sub> solution was used. The salt solution was concurrently added until 240 mL of the AgNO<sub>3</sub> solution had been added, then a new salt solution of 2.5 M NaBr, 0.04 M KI to which 0.45 g per L of bromine was added was used to maintain a pBr of 1.44 throughout the rest of the precipitation. The total making time of the emulsion was 194 min. The emulsion was cooled to 40° C. and ultrafiltered to a pBr of 3.26. Then 12.4 g per mole silver of bone gelatin (methionine content ~55 micromole per g gelatin) was added.

The resulting tabular grain emulsion was similar to Emulsion SI in the measured grain parameters of average ECD, thickness, and proportion of tabular grains as a percentage of total grain projected area.

#### Epitaxy

Epitaxy was deposited on the grains of each of Emulsions S1 and G1 by the following procedure: A vigorously stirred

1.0 mole aliquot of the emulsion was adjusted to a pAg of 7.59 at 40° C. by the addition of 0.25 M AgNO<sub>3</sub> solution. Then 5 mL of a 1M KI solution was added followed by 11 mL of a 3.77 M NaCl solution. Then the blue spectral sensitizing dye, anhydro-5,5'-dichloro-3,3'-bis(3-sulfonylpropyl)thiacyanine hydroxide, triethylammonium salt, was added in the form of a gelatin-dye dispersion in an amount of 80% of the saturation coverage of the grains' surfaces. After stirring for 25 min, 84 mL of a 0.25 M NaCl solution and 84 mL of a 0.25 M NaBr solution were added followed by 8 mmole of an AgI fine grain (~0.05  $\mu$ m) emulsion. To this mixture with vigorous stirring was added 0.5 M AgNO<sub>3</sub> at 76 mL per min for 1.1 min.

Electron microscopy analysis of the resulting emulsions showed the tabular grains had epitaxial deposits located primarily at the tabular grain comers and edges. As formulated these deposits had a nominal halide composition of 42 M % chloride, 42 M % bromide, and 16 M % iodide, based on silver.

#### Chemical Sensitization

To each of Emulsions 1S and 1G with epitaxy were added with stirring at 40° C. solutions of (amount per mole silver) NaSCN (0.925 mmole), 1,3-dicarboxymethyl-1,3-dimethyl-2-thiourea, (the optimized level for each emulsion was found to be the same, 7.8 micromole), bis(1,4,5-trimethyl-1,2,4-triazolium-3-thiolate) gold(I) tetrafluoroborate (the optimized level for each emulsion was found to be the same, 1.5 micromole), 3-{3-[(methylsulfonyl)amino]-3-oxopropyl} benzothiazolium tetrafluoroborate (the optimized level for each emulsion was found to be the same, 81 micromole). The emulsions were then heated at 50° C. for 10 minutes, cooled to 40° C., then sequentially 1-(3-acetamidophenyl)-5-mercaptopetrazole (0.489 mmole), FED 2 (2.8 micromole), and 4-hydroxy-6-methyl-1,3,3a,7-tetraazaindene (10 mmole) were added.

#### Performance Comparison

Each of sensitized Emulsions S1 and G1 were coated on clear acetate support having an antihalation layer on the opposite side. The coatings had laydowns of 1.08 g/m<sup>2</sup> silver, 1.62 g/m<sup>2</sup> yellow dye-forming coupler, 3.2 g/m<sup>2</sup> gelatin and surfactant. A solution of gelatin and bis(vinylsulfonylmethyl)ether were overcoated at 0.9 g/m<sup>2</sup> gelatin and 72 mg/m<sup>2</sup> hardener, respectively. Each of the film coatings were exposed for 0.01 sec to a 5500 K color temperature tungsten light source filtered through a 2B Kodak Wratten filter and a 0 to 4 density step tablet. The exposed film coatings were processed using the Kodak Flexicolor™ C-41 color negative film process.

Minimum density ( $D_{min}$ ), Gamma and Speed are compared below in Table II. Speed is reported as relative log speed, where a speed difference of 1 relative log speed difference is equal to an exposure difference of 0.01 log E, where E represents exposure in lux-seconds. Speed was measured on the characteristic curve at the intersection of the extrapolated straight line portion of the characteristic curve with the straight line extrapolation of the  $D_{min}$  segment of the characteristic curve. Gamma is the slope of the straight line portion of the characteristic curve.

TABLE II

| Emulsion     | $D_{min}$ | Gamma | Speed |
|--------------|-----------|-------|-------|
| S1 (example) | 0.13      | 1.80  | 130   |
| G1 (control) | 0.10      | 1.97  | 106   |

From Table II it is apparent that the cationic starch peptized high bromide {111} tabular grain Emulsion S1 was nearly a

stop (0.30 log E) faster in speed than the comparable gelatin peptized Emulsion G1. A stop speed advantage translates to a doubling of speed. Specifically, the 24 higher relative log speed units of Emulsion S1 amounts of a speed advantage of 0.24 log E over Emulsion G1.

### Example 2

In Example 1 the large speed advantage of Emulsion S1 over Emulsion G1 is in part attributable to the known speed advantage for substituting a cationic starch peptizer for gelatin and in part unexpected. This example has as its purpose to ascertain the extent of the speed advantage that results from substituting cationic starch peptizer for gelatino-peptizer, with no FED sensitizer present.

Emulsions S1 and G1 were remade as Emulsions S2 and G2 with these modifications: The FED sensitizer was omitted and the bromine oxidizing agent used to control elevated fog generated by FED sensitizer was also omitted. Repeating the performance comparison of Example 1, the following performance characteristics were noted:

TABLE III

| Emulsion    | D <sub>min</sub> | Gamma | Speed |
|-------------|------------------|-------|-------|
| S2 (no FED) | 0.11             | 1.85  | 107   |
| G2 (no FED) | 0.10             | 0.71  | 100   |

The speeds reported in Tables II and III are all referenced to Emulsion G2. From Table III it is apparent that the substitution of cationic starch peptizer for gelatin produces a speed advantage, previously known in the art, of 0.07 log E. Subtracting this expected speed advantage from the 0.24 log E speed advantage observed for Emulsion S1, indicates an unexpected added speed advantage when FED sensitizer is present of 0.17 log E (approximately one half stop, 0.15 log E).

### Example 3

This example has as its purpose to demonstrate the advantage in minimum density attributable to the presence of the oxidizing agent during grain precipitation in Emulsion S1.

An emulsion satisfying the requirements of the invention, Emulsion S3, was precipitated similarly as Emulsion S1, except that the bromine oxidizing agent added during precipitation was omitted. In all other respects Example 1 was repeated. The reported grain parameters of Emulsions S1 and S3 were similar. The performance of Emulsions S1, G1 and S2 are compared in Table IV.

TABLE IV

| Emulsion     | D <sub>min</sub> | Gamma | Speed |
|--------------|------------------|-------|-------|
| S1 (example) | 0.13             | 1.80  | 130   |
| G1 (control) | 0.10             | 1.97  | 106   |
| S3 (example) | 0.21             | 1.80  | 126   |

From Table IV it is apparent that, in the absence of the bromine oxidizing agent, a large unexpected speed advantage remains in evidence attributable to the combination of cationic starch peptizer and FED sensitizer. The disadvantage of omitting the oxidizing agent is a 0.11 increase in D<sub>min</sub>. This increase in minimum density, can be accommodated in some applications, such as color negative imaging, but would be objectionable in a color print, for instance. Hence, use of the oxidizing agent is preferred, but not required.

### Example 4

This example has as its purpose to demonstrate that delaying oxidizing agent addition until after precipitation is effective.

5 Example 1 was repeated as applied to Emulsion S1, but with the difference that bromine was absent from the emulsion during precipitation, but was added subsequent to precipitation by the following procedure:

10 Example Emulsion S4 was prepared similarly to that of Emulsion S1, except that no bromine was used before or during the precipitation. After the precipitation was complete, 28 nL of saturated bromine water (~0.013 mole) was added to the stirred emulsion at 40° C. maintaining the pH at 5.0 with dilute NaOH solution. (The reaction was over within 2 min after the bromine water addition, as indicated by the amount of NaOH that was needed to maintain the pH at 5.0.) The emulsion was ultrafiltered.

15 The measured grain parameters of Example Emulsions S1 and S4 were identical. The performance of Emulsions S1, S3 and S4 are compared in Table V.

TABLE V

| Emulsion          | D <sub>min</sub> | Gamma | Speed |
|-------------------|------------------|-------|-------|
| S1 (pptn Br)      | 0.13             | 1.80  | 130   |
| S3 (no Br)        | 0.21             | 1.80  | 126   |
| S4 (post pptn Br) | 0.16             | 1.69  | 130   |

20 From Table V it is apparent that bromine added following precipitation (pptn) is effective in limiting minimum density, although not as effective a bromine added during precipitation. The unexpected speed advantage of employing a cationic starch peptizer in combination with a FED sensitizer is observed in each of Emulsions S1, S3 and S4.

### Example 5

25 This example has as its purpose to demonstrate the additional speed enhancement that can be realized by blending light scattering particles with the starch peptized FED sensitized high bromide {111} tabular grain emulsions.

30 The procedure of Example 1 was followed, except that the emulsion layer coatings were varied by increasing the coating coverage of gelatin to 4.32 g/m<sup>2</sup>. Additionally, in all but one coating, light scattering silver halide grains were incorporated in a coating coverage of 0.108 g/m<sup>2</sup>.

35 The results are summarized in Table VI:

| Coating | ESD, $\mu\text{m}$ | Content                                  | Particle         |       |       | Relative Speed |
|---------|--------------------|------------------------------------------|------------------|-------|-------|----------------|
|         |                    |                                          | D <sub>min</sub> | Gamma | Speed |                |
| C5      | none               | none                                     | 0.22             | 1.87  | 100   |                |
| E5a     | 0.495              | AgBr                                     | 0.22             | 1.90  | 109   |                |
| E5b     | 0.60               | AgI <sub>0.002</sub> Cl <sub>0.998</sub> | 0.27             | 1.96  | 141   |                |
| E5c     | 0.38               | AgCl                                     | 0.33             | 2.29  | 121   |                |

40 55 The addition of each of AgBr, AgI<sub>0.002</sub>Cl<sub>0.998</sub> and AgCl grains increases speed and contrast. The particles that are free of chloride offer the advantage that the speed enhancement does not also increase minimum density.

60 The invention has been described in detail with particular reference to certain preferred embodiments thereof, but it will be understood that variations and modifications can be effected within the spirit and scope of the invention.

65 What is claimed is:

1. A photographic element comprised of a support and coated on the support at least one emulsion layer comprised of

- (a) radiation-sensitive silver halide grains,  
 (b) sensitizer for the radiation-sensitive silver halide grains,  
 (c) hydrophilic colloid vehicle, including peptizer for the radiation-sensitive silver halide grains, and  
 (d) light scattering particles,  
 wherein

(a) the radiation-sensitive silver halide grains include tabular grains (1) having an aspect ratio of at least 2.0, (2) having {111} major faces, (3) containing greater than 50 mole percent bromide, based on silver, and (4) accounting for greater than 50 percent total grain projected area,  
 (b) the sensitizer includes a fragmentable electron donating sensitizer,  
 (c) the peptizer is a water dispersible cationic starch, and  
 (d) the light scattering particles have aspect ratios of less than 1.5 and can be dissolved for removal from the emulsion layer.

2. A photographic element according to claim 1 wherein the fragmentable electron donating sensitizer contains a moiety for promoting adsorption to silver halide grain surfaces.

3. A photographic element according to claim 1 wherein the radiation-sensitive silver halide grains include tabular grains containing greater than 70 mole percent bromide, based on silver, and account for greater than 70 percent of total grain projected area.

4. A photographic element according to claim 3 wherein the radiation-sensitive silver halide grains include tabular grains containing at least 90 mole percent bromide, based on silver, and account for at least 90 percent of total grain projected area.

5. A photographic element according to claim 1 wherein the fragmentable electron donating sensitizer fragments upon oxidation to provide a radical that exhibits an oxidation potential equal to or more negative than -0.7 volt.

6. A photographic element according to claim 1 wherein the cationic starch is a water dispersible oxidized cationic starch.

7. A photographic element according to claim 1 wherein the cationic starch contains  $\alpha$ -D-glucopyranose repeating units and, on average, at least 1 percent of the  $\alpha$ -D-glucopyranose repeating units are ring opened by oxidation.

8. A photographic element according to claim 1 wherein the light scattering particles are removable during photographic processing.

9. A photographic element according to claim 8 wherein the light scattering particles are removable under the following conditions of photographic processing:

| step    | time  | bath | temperature |
|---------|-------|------|-------------|
| develop | 3'15" | D    | 37.8° C.    |
| bleach  | 4'    | B    | 37.8° C.    |
| wash    | 3'    | W    | 35.5° C.    |
| fix     | 4'    | F    | 37.8° C.    |
| wash    | 3'    | W    | 35.5° C.    |
| rinse   | 1'    | R    | 37.8° C.    |

wherein

'represents minutes;

"represents seconds;

bath D exhibits the following composition:

|                                |          |
|--------------------------------|----------|
| water                          | 800.0 mL |
| potassium carbonate, anhydrous | 34.30 g  |

-continued

|                                                   |         |
|---------------------------------------------------|---------|
| potassium bicarbonate                             | 2.32 g  |
| sodium sulfite, anhydrous                         | 0.38 g  |
| sodium metabisulfite                              | 2.96 g  |
| potassium iodide                                  | 1.20 mg |
| sodium bromide                                    | 1.31 g  |
| diethylenetriaminepentaacetic acid                | 8.43 g  |
| pentasodium salt (40% soln)                       |         |
| hydroxylamine sulfate                             | 2.41 g  |
| N-(4-amino-3-methylphenyl)-N-ethyl-2-aminoethanol | 4.52 g  |
| water to make                                     | 1.0 L   |
| pH @ 26.7° C. 10.00 +/- 0.05;                     |         |

bath B represents the following composition:

|                                                 |          |
|-------------------------------------------------|----------|
| water                                           | 500.0 mL |
| 1,3-propylenediamine tetra-acetic acid          | 37.4 g   |
| 57% ammonium hydroxide                          | 70.0 mL  |
| acetic acid                                     | 80.0 mL  |
| 2-hydroxy-1,3-propylenediamine tetraacetic acid | 0.8 g    |
| ammonium bromide                                | 25.0 g   |
| ferric nitrate nonahydrate                      | 44.85 g  |
| water to make                                   | 1.0 L    |
| pH 4.75;                                        |          |

bath F represents the following composition:

|                                     |          |
|-------------------------------------|----------|
| water                               | 500.0 mL |
| ammonium thiosulfate (58% solution) | 214.0 g  |
| (ethylenedinitrilo)tetraacetic acid | 1.29 g   |
| disodium salt, dihydrate            |          |
| sodium metabisulfite                | 11.0 g   |
| sodium hydroxide (50% solution)     | 4.70 g   |
| water to make                       | 1.0 L    |
| pH at 26.7° C. 6.5 +/- 0.15;        |          |

bath R represents the following composition:

|                                                                      |            |
|----------------------------------------------------------------------|------------|
| water                                                                | 900.0 mL   |
| 0.5% aqueous p-tertiary-octyl-( $\alpha$ -phenoxypropylethyl)alcohol | 3.0 mL     |
| water to make                                                        | 1.0 L; and |

bath W represents water.

10. A photographic element according to claim 1 wherein the vehicle is comprised of gelatin or a gelatin derivative binder and the light scattering particles have a refractive index of at least 1.9.

11. A photographic element according to claim 10 wherein the particles have a refractive index of at least 2.0.

12. A photographic element according to claim 1 wherein the light scattering particles have a mean equivalent spherical diameter in the range of from 0.1 to 1.0  $\mu$ m.

13. A photographic element according to claim 12 wherein the light scattering particles have a mean equivalent spherical diameter in the range of from 0.2 to 0.8  $\mu$ m.

14. A photographic element according to claim 1 wherein the light scattering particles have a coefficient of variation of less than 20 percent.

15. A photographic element according to claim 1 wherein the light scattering particles are cubic, octahedral, or tetradecahedral particles, including forms in which edge and corner rounding has occurred.

16. A photographic element according to any one of claims 1 to 15 inclusive comprised of

a transparent film support, blue, green and red recording layer units coated on the support for recording exposures to the blue, green and red regions of the visible spectrum, respectively, at least one of the recording layer units containing said emulsion.